



US008927472B2

(12) **United States Patent**  
**Cholli et al.**

(10) **Patent No.:** **US 8,927,472 B2**  
(b4) **Date of Patent:** **Jan. 6, 2015**

(54) **LUBRICANT OIL COMPOSITIONS**

(75) Inventors: **Ashok L. Cholli**, Chelmsford, MA (US);  
**Ashish Dhawan**, Lowell, MA (US);  
**Rajesh Kumar**, Dracut, MA (US);  
**Vijayendra Kumar**, Dracut, MA (US);  
**Suizhou Yang**, Lowell, MA (US);  
**Taizoon Canteenwala**, Lowell, MA (US)

(73) Assignee: **Polnox Corporation**, Lowell, MA (US)

(\*) Notice: Subject to any disclaimer, the term of this patent is extended or adjusted under 35 U.S.C. 154(b) by 0 days.

(21) Appl. No.: **13/469,813**

(22) Filed: **May 11, 2012**

(65) **Prior Publication Data**

US 2013/0130955 A1 May 23, 2013

**Related U.S. Application Data**

(63) Continuation of application No. 13/165,372, filed on Jun. 21, 2011, now abandoned, which is a continuation of application No. 11/606,785, filed on Nov. 30, 2006, now abandoned.

(60) Provisional application No. 60/742,150, filed on Dec. 2, 2005.

(51) **Int. Cl.**

**C10M 133/04** (2006.01)  
**C10M 141/00** (2006.01)  
**C10M 157/00** (2006.01)  
**C10M 161/00** (2006.01)

(52) **U.S. Cl.**

CPC ..... **C10M 133/04** (2013.01); **C10M 141/00** (2013.01); **C10M 2219/087** (2013.01); **C10M 2215/064** (2013.01); **C10M 2215/062** (2013.01); **C10M 2207/08** (2013.01); **C10M 2217/04** (2013.01); **C10M 2223/049** (2013.01); **C10M 2207/024** (2013.01); **C10M 2207/026** (2013.01); **C10M 2207/289** (2013.01); **C10N 2230/10** (2013.01); **C10M 2223/045** (2013.01); **C10M 2209/04** (2013.01); **C10N 2260/00** (2013.01); **C10M 2217/046** (2013.01); **C10M 2217/041** (2013.01); **C10M 157/00** (2013.01); **C10M 2215/14** (2013.01); **C10M 2215/082** (2013.01); **C10M 2207/284** (2013.01); **C10M 161/00** (2013.01)

USPC ..... **508/560**; 508/192

(58) **Field of Classification Search**

USPC ..... 508/192, 560

See application file for complete search history.

(56) **References Cited**

## U.S. PATENT DOCUMENTS

3,116,305 A 12/1963 Morris et al.  
3,294,836 A 12/1966 Peterson et al.  
3,441,545 A 4/1969 Blatz et al.

3,459,704 A 8/1969 Peterson et al.  
3,557,245 A 1/1971 Phillips et al.  
3,632,785 A 1/1972 Bornstein  
3,645,970 A 2/1972 Kleiner  
3,649,667 A 3/1972 Song et al.  
3,655,831 A 4/1972 Friedman  
3,870,680 A 3/1975 Schurdak  
3,907,939 A 9/1975 Robin et al.  
3,953,402 A 4/1976 Kline  
3,965,039 A 6/1976 Chaplits et al.  
3,983,091 A 9/1976 Gloth et al.  
3,994,828 A 11/1976 Zaffaroni  
3,996,160 A 12/1976 Dale et al.  
3,996,198 A 12/1976 Wang et al.  
4,054,676 A 10/1977 Weinshenker et al.  
4,094,857 A 6/1978 Wolfe, Jr.  
4,096,319 A 6/1978 Willette et al.  
4,097,464 A 6/1978 Kline  
4,098,829 A 7/1978 Weinshenker et al.  
4,107,144 A 8/1978 Russell et al.  
4,136,055 A 1/1979 Lyons  
4,202,816 A 5/1980 Moser et al.  
4,205,151 A 5/1980 Dale et al.  
4,213,892 A 7/1980 Scott  
4,219,453 A 8/1980 Sakurai et al.  
4,267,358 A 5/1981 Hechenbleikner et al.  
4,281,192 A 7/1981 Jaquet et al.  
4,283,572 A 8/1981 Klicker  
4,317,933 A 3/1982 Parker  
4,341,879 A 7/1982 Sugio et al.  
4,355,148 A 10/1982 Layer et al.  
4,377,666 A 3/1983 Farrar  
4,380,554 A 4/1983 Serres, Jr.  
4,447,657 A 5/1984 Firth et al.

(Continued)

## FOREIGN PATENT DOCUMENTS

|    |               |        |
|----|---------------|--------|
| CS | 111291        | 6/1964 |
| DE | 197 47 644 A1 | 5/1999 |

(Continued)

## OTHER PUBLICATIONS

<http://www.machinerylubrication.com/Read/1028/Oxidation-Lubricant> (Mar. 29, 2010, pp. 1-7).  
Akkara, J.A., et al., "Hematin-Catalyzed Polymerization of Phenol Compounds," *Macromolecules*, 33(7):2377-2382 (2000).  
Akkara, J.A., et al., "Synthesis and Characterization of Polymers Produced by Horseradish Peroxidase in Dioxane," *J. of Polymer Science: Part A: Polymer Chemistry*, 29(11):1561-1574 (1991).

(Continued)

Primary Examiner — James Goloboy

(74) Attorney, Agent, or Firm — Hamilton, Brook, Smith & Reynolds, P.C.

(57) **ABSTRACT**

Compositions comprise first antioxidants and first additives, such as, a surface additives, performance enhancing additives and lubricant protective additives and optionally second additives and/or second antioxidants. The compositions are useful to improve lubricants, lubricant oils and other lubricant materials. The compositions and methods generally provide longer shelf lives, increased oxidative resistance, improved quality and/or enhanced performance to lubricants or lubricant oils.

12 Claims, No Drawings

(56)

## References Cited

U.S. PATENT DOCUMENTS

| References Cited |    | U.S. PATENT DOCUMENTS |                    | FOREIGN PATENT DOCUMENTS |            |         |                       |  |
|------------------|----|-----------------------|--------------------|--------------------------|------------|---------|-----------------------|--|
| 4,465,871        | A  | 8/1984                | Firth et al.       | 7,956,153                | B2         | 6/2011  | Cholli et al.         |  |
| 4,510,296        | A  | 4/1985                | Hergenrother       | 8,008,423                | B2         | 8/2011  | Kumar et al.          |  |
| 4,511,491        | A  | 4/1985                | Ishii et al.       | 8,039,673                | B2         | 10/2011 | Cholli et al.         |  |
| 4,634,728        | A  | 1/1987                | Dunski et al.      | 8,080,689                | B2         | 12/2011 | Kumar                 |  |
| 4,690,995        | A  | 9/1987                | Keskey et al.      | 8,242,230                | B2         | 8/2012  | Cholli et al.         |  |
| 4,761,247        | A  | 8/1988                | Rei et al.         | 8,252,884                | B2         | 8/2012  | Kumar et al.          |  |
| 4,824,929        | A  | 4/1989                | Arimatsu et al.    | 8,481,670                | B2         | 7/2013  | Kumar et al.          |  |
| 4,849,503        | A  | 7/1989                | Cotter et al.      | 8,598,382                | B2         | 12/2013 | Cholli et al.         |  |
| 4,855,345        | A  | 8/1989                | Rosenberger et al. | 8,691,933                | B2         | 4/2014  | Kumar et al.          |  |
| 4,857,596        | A  | 8/1989                | MacLeay et al.     | 8,710,266                | B2         | 4/2014  | Kumar et al.          |  |
| 4,870,214        | A  | 9/1989                | Mina et al.        | 2001/0041203             | A1         | 11/2001 | Uno et al.            |  |
| 4,894,263        | A  | 1/1990                | Dubois et al.      | 2002/0007020             | A1         | 1/2002  | Higahimura et al.     |  |
| 4,897,438        | A  | 1/1990                | Kikuchi et al.     | 2002/0128493             | A1         | 9/2002  | Romanczyk, Jr. et al. |  |
| 4,900,671        | A  | 2/1990                | Pokora et al.      | 2002/0143025             | A1         | 10/2002 | Pratt et al.          |  |
| 4,925,591        | A  | 5/1990                | Nakauchi et al.    | 2002/0183470             | A1         | 12/2002 | Tripathy et al.       |  |
| 4,968,759        | A  | 11/1990               | Kikuchi et al.     | 2003/0030033             | A1         | 2/2003  | Duyck et al.          |  |
| 4,977,004        | A  | 12/1990               | Bettle, III et al. | 2003/0078346             | A1         | 4/2003  | Nakamura et al.       |  |
| 4,981,917        | A  | 1/1991                | MacLeay et al.     | 2003/0091837             | A1         | 5/2003  | Aoki                  |  |
| 4,994,628        | A  | 2/1991                | Goddard et al.     | 2003/0176620             | A1         | 9/2003  | Romanczyk, Jr. et al. |  |
| 5,013,470        | A  | 5/1991                | Benfaremo          | 2003/0191242             | A1         | 10/2003 | Zedda et al.          |  |
| 5,017,727        | A  | 5/1991                | Olivier            | 2003/0229196             | A1         | 12/2003 | Bratt et al.          |  |
| 5,082,358        | A  | 1/1992                | Tabata et al.      | 2003/0230743             | A1         | 12/2003 | Cholli et al.         |  |
| 5,102,962        | A  | 4/1992                | Kikuchi et al.     | 2004/0015021             | A1         | 1/2004  | Adams et al.          |  |
| 5,117,063        | A  | 5/1992                | Stern et al.       | 2004/0164279             | A1         | 8/2004  | Stevenson et al.      |  |
| 5,143,828        | A  | 9/1992                | Akkara et al.      | 2004/0180994             | A1         | 9/2004  | Pearson et al.        |  |
| 5,155,153        | A  | 10/1992               | Neri et al.        | 2004/0186167             | A1         | 9/2004  | Dou et al.            |  |
| 5,185,391        | A  | 2/1993                | Stokich, Jr.       | 2004/0186214             | A1         | 9/2004  | Li et al.             |  |
| 5,185,407        | A  | 2/1993                | Wong               | 2004/0198875             | A1         | 10/2004 | Kaprinidis et al.     |  |
| 5,188,953        | A  | 2/1993                | Johnson et al.     | 2004/0214935             | A1         | 10/2004 | Cholli et al.         |  |
| 5,191,008        | A  | 3/1993                | Frost et al.       | 2005/0170978             | A1         | 8/2005  | Migdal et al.         |  |
| 5,196,142        | A  | 3/1993                | Mollet et al.      | 2005/0209379             | A1         | 9/2005  | Botkin et al.         |  |
| 5,206,303        | A  | 4/1993                | Tse et al.         | 2005/0238789             | A1         | 10/2005 | Cholli et al.         |  |
| 5,207,939        | A  | * 5/1993              | Farng et al.       | 2005/0242328             | A1         | 11/2005 | Baranski              |  |
| 5,274,060        | A  | 12/1993               | Schadeli           | 2006/0029706             | A1         | 2/2006  | Cholli et al.         |  |
| 5,278,055        | A  | 1/1994                | Cyrus, Jr. et al.  | 2006/0040833             | A1         | 2/2006  | Al-Akhdar et al.      |  |
| 5,304,589        | A  | 4/1994                | Davidson et al.    | 2006/0041087             | A1         | 2/2006  | Cholli                |  |
| 5,320,889        | A  | 6/1994                | Bettle, III        | 2006/0041094             | A1         | 2/2006  | Cholli                |  |
| 5,449,715        | A  | 9/1995                | Plochocka et al.   | 2006/0128929             | A1         | 6/2006  | Yang et al.           |  |
| 5,498,809        | A  | 3/1996                | Emert et al.       | 2006/0128930             | A1         | 6/2006  | Dhawan et al.         |  |
| RE35,247         | E  | 5/1996                | Cyrus, Jr. et al.  | 2006/0128931             | A1         | 6/2006  | Kumar et al.          |  |
| 5,516,856        | A  | 5/1996                | Sanchez            | 2006/0128939             | A1         | 6/2006  | Kumar et al.          |  |
| 5,541,091        | A  | 7/1996                | Wheeler et al.     | 2006/0154818             | A1         | 7/2006  | Destro et al.         |  |
| 5,565,300        | A  | 10/1996               | Uenishi et al.     | 2006/0189820             | A1         | 8/2006  | Rehm et al.           |  |
| 5,574,118        | A  | 11/1996               | Olivier            | 2006/0189824             | A1         | 8/2006  | Kumar et al.          |  |
| 5,652,201        | A  | * 7/1997              | Papay et al.       | 2006/0202227             | A1         | 9/2006  | Shiraki               |  |
| 5,739,341        | A  | 4/1998                | Dubs et al.        | 2006/0233741             | A1         | 10/2006 | Kumar et al.          |  |
| 5,834,544        | A  | 11/1998               | Lin et al.         | 2007/0010632             | A1         | 1/2007  | Kaplan et al.         |  |
| 5,837,798        | A  | 11/1998               | Hutchings et al.   | 2007/0106059             | A1         | 5/2007  | Cholli et al.         |  |
| 5,869,592        | A  | 2/1999                | Gagne et al.       | 2007/0135539             | A1         | 6/2007  | Cholli et al.         |  |
| 5,911,937        | A  | 6/1999                | Hekal              | 2007/0149660             | A1         | 6/2007  | Kumar et al.          |  |
| 5,994,498        | A  | 11/1999               | Tripathy et al.    | 2007/0154430             | A1         | 7/2007  | Cholli et al.         |  |
| 6,018,018        | A  | 1/2000                | Samuelson et al.   | 2007/0154608             | A1         | 7/2007  | Cholli et al.         |  |
| 6,046,263        | A  | 4/2000                | Rasberger et al.   | 2007/0154720             | A1         | 7/2007  | Cholli et al.         |  |
| 6,096,695        | A  | 8/2000                | Lam et al.         | 2007/0161522             | A1         | 7/2007  | Cholli et al.         |  |
| 6,096,859        | A  | 8/2000                | Akkara et al.      | 2008/0249335             | A1         | 10/2008 | Cholli et al.         |  |
| 6,150,491        | A  | 11/2000               | Akkara             | 2008/0293856             | A1         | 11/2008 | Kumar et al.          |  |
| 6,232,314        | B1 | 5/2001                | Jarrott et al.     | 2008/0311065             | A1         | 12/2008 | Cholli                |  |
| 6,342,549        | B1 | 1/2002                | Hirose et al.      | 2009/0184294             | A1         | 7/2009  | Cholli et al.         |  |
| 6,444,450        | B2 | 9/2002                | Akkara et al.      | 2011/0040125             | A1         | 2/2011  | Kumar et al.          |  |
| 6,646,035        | B2 | 11/2003               | Koch et al.        | 2011/0282098             | A1         | 11/2011 | Cholli et al.         |  |
| 6,723,815        | B2 | 4/2004                | Callaghan et al.   | 2012/0004150             | A1         | 1/2012  | Cholli et al.         |  |
| 6,743,525        | B2 | 6/2004                | Bernsten et al.    | 2012/0071596             | A1         | 3/2012  | Kumar et al.          |  |
| 6,770,785        | B1 | 8/2004                | Desai et al.       | 2012/0123145             | A1         | 5/2012  | Cholli et al.         |  |
| 6,794,480        | B2 | 9/2004                | Goto et al.        | 2012/0142968             | A1         | 6/2012  | Kumar et al.          |  |
| 6,800,228        | B1 | 10/2004               | Semen              | 2013/0041171             | A1         | 2/2013  | Cholli et al.         |  |
| 6,828,364        | B2 | 12/2004               | Gugumus            | 2013/0072586             | A1         | 3/2013  | Kumar et al.          |  |
| 6,846,859        | B2 | 1/2005                | Coffy et al.       | 2014/0011901             | A1         | 1/2014  | Kumar et al.          |  |
| 7,132,496        | B2 | 11/2006               | Kerres et al.      | 2014/004880              | A1         | 1/2014  | Cholli et al.         |  |
| 7,169,844        | B2 | 1/2007                | Inokami            | DE                       | 198 43 875 | A1      | 3/2000                |  |
| 7,205,350        | B2 | 4/2007                | Thibaut            | EP                       | 0 181 023  | A1      | 5/1986                |  |
| 7,223,432        | B2 | 5/2007                | Cholli et al.      | EP                       | 0 289 077  | A2      | 11/1988               |  |
| 7,262,319        | B2 | 8/2007                | Rehm et al.        | EP                       | 0 358 157  |         | 3/1990                |  |
| 7,705,176        | B2 | 4/2010                | Cholli et al.      | EP                       | 0 404 039  | A1      | 12/1990               |  |
| 7,705,185        | B2 | 4/2010                | Kumar et al.       | EP                       | 0 618 203  | A1      | 10/1994               |  |
| 7,902,317        | B2 | 3/2011                | Kumar et al.       | EP                       | 0 688 805  | A1      | 12/1995               |  |
|                  |    |                       |                    | EP                       | 1 067 144  | A1      | 1/2001                |  |

## FOREIGN PATENT DOCUMENTS

(56)

## References Cited

## FOREIGN PATENT DOCUMENTS

EP 1 468 968 A1 10/2004  
 FR 2 183 973 12/1973  
 GB 1042639 8/1964  
 GB 1 283 103 7/1972  
 GB 1 320 169 6/1973  
 GB 1 372 042 10/1974  
 GB 1 389 442 4/1975  
 GB 1 469 245 4/1977  
 GB 1 482 649 8/1977  
 JP 69002715 B 1/1966  
 JP 43016392 B4 7/1968  
 JP 43018453 8/1968  
 JP 44024274 10/1969  
 JP 44028850 11/1969  
 JP 45 2980 1/1970  
 JP 45-2980 1/1970  
 JP 49 29339 3/1974  
 JP 57085366 A 5/1982  
 JP 59025814 2/1984  
 JP 59197447 11/1984  
 JP 60-199832 10/1985  
 JP 05 199858 8/1993  
 JP 06135876 A 5/1994  
 JP 06 247959 9/1994  
 JP 08027226 A 1/1996  
 JP 09262069 10/1997  
 JP 09 328519 12/1997  
 JP 09 328521 12/1997  
 JP 9322784 A 12/1997  
 JP 11-80063 3/1999  
 JP 11-158103 6/1999  
 JP 2003138258 5/2003  
 NL 7 905 000 3/1980  
 WO WO 92/20734 11/1992  
 WO WO 00/39064 7/2000  
 WO WO 01/18125 A1 3/2001  
 WO WO 01/48057 A1 7/2001  
 WO WO 02/079130 A1 10/2002  
 WO WO 03/087260 A1 10/2003  
 WO WO 03/102004 A1 12/2003  
 WO WO 2004/024070 A2 3/2004  
 WO WO 2004/050795 A2 6/2004  
 WO WO 2005/025513 A2 3/2005  
 WO WO 2005/025646 A2 3/2005  
 WO WO 2005/060500 A2 7/2005  
 WO WO 2005/070974 A2 8/2005  
 WO WO 2005/071005 A1 8/2005  
 WO WO 2006/018403 A1 2/2006  
 WO WO 2006/060801 A2 6/2006  
 WO WO 2006/104957 A2 10/2006  
 WO WO 2008/005358 A2 1/2008

## OTHER PUBLICATIONS

- Al-Malaika, S and Suharty, N., "Reactive Processing of Polymers: Mechanisms of Grafting Reactions of Functional Antioxidants on Polyolefins in the Presence of a Coagent," *Polymer Degradation and Stability* 49: 77-89 (1995).
- Armenol, E., et al., "Acid Zeolites as Catalysts in Organic Reactions, tert-Butylation of Anthracene, Naphthalene and Thianthrene," *Appl. Catal. A* 149:411-423 (1997).
- Ayyagari, M.S., et al., "Controlled Free-Radical Polymerization of Phenol Derivatives by Enzyme-Catalyzed Reactions in Organic Solvents," *Macromolecules*, 28(15):5192-5197 (1995).
- Badamali, S.K., et al., "Influence of Aluminium Sources on the Synthesis and Catalytic Activity of Mesoporous AIMCM-41 Molecular Sieves," *Catal. Today* 63:291-295 (2000).
- Belyaev, A., et al., "Structure-Activity Relationship of Diaryl Phosphonate Esters as Potent Irreversible Dipeptidyl Peptidase IV Inhibitors," *J. Med. Chem.*, 42:1041-1052 (1999).
- Blokhin, Y.I., et al., "Phosphorylation of Dihydric Phenols with Amides of Phosphorous Acid," *Russian Chem. Bulletin*, 45(9):2250-2251 (1996).
- Bruno, F.F., et al., "Enzymatic Template Synthesis of Polyphenol," *Materials Research Society Symposium Proceedings* vol. 600, *Electroactive Polymers (EAP)*:255-259 (1999).
- Chandra, K.G. and Sharma, M.M., "Alkylation of Phenol with MTBE and Other tert-butylethers:Cation Exchange Resins as Catalysts," *Catal. Lett.* 19(4):309-317 (1993).
- Circ-Marjanovic, et al., Chemical Oxidative Polymerization of Aminodiphenylamines, *Journal of Physical Chemistry B*, 112, 23: 6976-6987 (2008).
- Coppinger, G.B., et al., "Photo-Fries Rearrangement of Aromatic Esters. Role of Steric and Electronic Factors" *J. of Phy. Chem.*, 70(11):3479-3489 (1966).
- Database Beilstein [online] Beilstein Institut Zur Förderung Der Chemischen Wissenschaften; XP002420027, Beilstein Registry No. 3517906.
- Database Beilstein [online] Beilstein Institut Zur Förderung Der Chemischen Wissenschaften; XP002420028, Beilstein Registry No. 5840042.
- Database Beilstein [online] Beilstein Institut Zur Förderung Der Chemischen Wissenschaften; XP002420029, Beilstein Registry No. 2311871.
- Database Beilstein [online] Beilstein Institut Zur Förderung Der Chemischen Wissenschaften; XP002420030, Beilstein Registry No. 8876646.
- Database Beilstein [online] Beilstein Institut Zur Förderung Der Chemischen Wissenschaften; XP002420031, Beilstein Registry No. 2271400.
- Database Beilstein [online] Beilstein Institut Zur Förderung Der Chemischen Wissenschaften; XP002420032, Beilstein Registry No. 2212095.
- Database Beilstein [online] Beilstein Institut Zur Förderung Der Chemischen Wissenschaften; XP002420033, Beilstein Registry No. 8941955.
- Database Beilstein [online] Beilstein Institut Zur Förderung Der Chemischen Wissenschaften; XP002420034, Database Accession No. 2312425.
- Database Beilstein [online] Beilstein Institut Zur Förderung Der Chemischen Wissenschaften; XP002420035, Beilstein Registry No. 905950.
- Database Beilstein [online] Beilstein Institut Zur Förderung Der Chemischen Wissenschaften; XP002420036, Beilstein Registry No. 2140308.
- Database Beilstein [online] Beilstein Institut Zur Förderung Der Chemischen Wissenschaften; XP002420037, Beilstein Registry No. 134886.
- Database Beilstein [online] Beilstein Institut Zur Förderung Der Chemischen Wissenschaften; XP002420038, Beilstein Registry No. 1961007.
- Database CA [online] Chemical Abstracts Service, Columbus, Ohio, US, XP-002429584, Database Accession No. 81:153647, Organic Phosphate Stabilizers for Polyamides and Polyurethanes, abstract, Minagawa, M. (1974).
- Database Caplus [online] Chemical Abstracts Service, Columbus, Ohio, US, XP-002387095, Database Accession No. 1981:572206, Effectiveness of Inhibitors in the Oxidation of Jet Fuel with an Initiator, abstract, Kovalev, et al.
- Devassy, B.M., et al., "Zirconia Supported Phosphotungstic Acid as an Efficient Catalyst for Resorcinol tert-Butylation and n-Heptane Hydroisomerization," *J. Mol. Catalysis A: Chemical* 221:113-119 (2004).
- Ding, et al., "Chemical Trapping Experiments Support a Cation-Radical Mechanism for the Oxidative Polymerization of Aniline," *Journal of Polymer Science, Part A: Polymer Chemistry*, vol. 37: 2569-2579 (1999).
- Dordick, J.S., "Enzymatic Catalysis in Monophasic Organic Solvents," *Enzyme Microb. Technol.*, 11(4):194-211 (1989).
- Dordick, J.S., et al., "Polymerization of Phenols Catalyzed by Peroxidase in Nonaqueous Media," *Biotechnology and Bioengineering*, XXX:31-36 (1987).
- English Abstract of Kovalev, G. I., et al., "Study of the Effectiveness of Inhibitors in Oxidation of Jet Fuel in a Closed Volume," *Deposited Doc.*, VINITI: 443-82 (1981).

(56)

## References Cited

## OTHER PUBLICATIONS

- English Abstract of Kovalev, G.I., et al., "Effectiveness of Inhibitors in the Oxidation of Jet Fuel With an Initiator," *J. Neftekhimiya (Petroleum Chemistry)*, 21(2): 287-298 (1981).
- Faber, K., "Biotransformations in Organic Chemistry," A Textbook, Fourth Completely Revised and Extended Edition, Springer-Verlag pp: 347-349 (1953).
- FS&T 821 "Antioxidant," [online], [retrieved on Oct. 29, 2002]. Retrieved from the Internet <URL: <http://class.fst.ohio-state.edu/fst821/>>.
- FS&T 821 "Food Lipids," [online], Oct. 2001 [retrieved on Oct. 29, 2002]. Retrieved from the Internet <URL: <http://class.fst.ohio-state.edu/fst821/>>.
- FST 821 "Course Schedule," [online], [retrieved on Oct. 29, 2002]. Retrieved from the Internet <URL: <http://class.fst.ohio-state.edu/fst821/>>.
- Hatayama, K., et al., "Anti-ulcer Effect of Isoprenyl Flavonoids. III.<sup>1)</sup> Synthesis and Anti-ulcer Activity of Metabolites of 2'-Carboxymethoxy-4,4'-bis(3-methyl-2-butenyloxy)chalcone<sup>2)</sup>," *Chemical & Pharmaceutical Bulletin*, 33(4), 1327-1333(Apr. 1985).
- Heidekum, A., et al., "Nafion/Silica Composite Material Reveals High Catalytic Potential in Acylation Reactions," *J. Catal.* 188:230-232 (1999).
- Hidalgo, M.E., et al., "Antioxidant Activity of Depsides and Depsidones," *Phytochemistry*, 37(6):1585-1587 (1994).
- Hofer, K., et al., "[[(Anilinooxalyl)amino]phenyl] Phosphite Stabilizers for Polypropylene," Chemical Abstracts Service, ZCPLUS, document No. 77:62780 (1972).
- Ikeda, R., et al., "Novel Synthetic Pathway to a Poly(phenylene oxide). Laccase-Catalyzed Oxidative Polymerization of Syringic Acid," *Macromolecules*, 29:3053-3054 (1996).
- International Search Report for related foreign application PCT/US2007/015177, mailed on Jun. 13, 2008.
- International Search Report for related foreign application PCT/US2005/044021, mailed on May 22, 2006.
- International Search Report for related foreign application PCT/US2005/044022, mailed on May 2, 2006.
- International Search Report for related foreign application PCT/US2005/044023, mailed on Nov. 3, 2006.
- International Search Report for related foreign application PCT/US2005/044019, mailed on Apr. 28, 2006.
- International Search Report for related foreign application PCT/US2005/025646, mailed on Mar. 13, 2006.
- International Search Report for related foreign application PCT/US2005/025513, mailed on Mar. 13, 2006.
- International Search Report for related foreign application PCT/US2006/006355, mailed on Jul. 31, 2006.
- International Search Report for related foreign application PCT/US2006/010985, mailed on Dec. 19, 2006.
- International Search Report for related foreign application PCT/US2006/042240, mailed on May 3, 2007.
- International Search Report for related foreign application PCT/US2006/042235, mailed on Apr. 27, 2007.
- International Search Report for related foreign application PCT/US2006/045929, mailed on Apr. 20, 2007.
- Ismail, M.N. and Wazzan, A.A., "Evaluation of New Thermal Stabilizers and Antifatigue Agents for Rubber Vulcanizates," *Polymer-Plastics Tech. and Eng.*, 45:751-758 (2006).
- Jayaprakasha, G.K., et al., "Antioxidant Activity of Grape Seed (*Vitis vinifera*) Extracts on Peroxidation Models in Vitro," *Food Chemistry*, 73:285-290 (2001).
- Jalianella, G. and Pilrma, I., "Synthesis of Poly(vinyl alcohol-co-vinyl gallate) by the Chemical Modification of Poly(vinyl alcohol)," *Polymer Bulletin* 18:385-389 (1987).
- Joossens, J., et al., "Diphenyl Phosphonate Inhibitors for the Urokinase-Type Plasminogen Activator: Optimization of the P4 Position," *J. Med. Chem.*, 49:5785-5793 (2006).
- Kamitori, Y., et al., "Silica Gel as an Effective Catalyst for the Alkylation of Phenols and Some Heterocyclic Aromatic Compounds," *J. Org. Chem.* 49: 4161-4165 (1984).
- Kazandjian, R.Z., et al., "Enzymatic Analyses in Organic Solvents," *Biotechnology and Bioengineering*, XXVIII:417-421 (1986).
- Khan, K.M., et al., "An Expedient Esterification of Aromatic Carboxylic Acids Using Sodium Bromate and Sodium Hydrogen Sulfite," *Tetrahedron* 59(29):5549-5554 (2003).
- Kim, T. H., et al., "Melt Free-Radical Grafting of Hindered Phenol Antioxidant onto Polyethylene," *J. Applied Polymer Science*, 77:2968-2973 (2000).
- Klibanov, A.M., et al., "Enzymatic Removal of Toxic Phenols and Anilines from Waste Waters," *J. of Applied Biochemistry*, 2(5):414-421 (1980).
- Koshchii, V.A., et al., "Alkylation of Phenol by Alcohols in the Presence of Aluminium Phenolate," *Org. Chem.* 24(7):1358-1361 (1988).
- Lalancette, J.M., et al., "Metals Intercalated in Graphite. II. The Friedel-Crafts Reactions with  $AlCl_3$ -Graphite," *Can. J. Chem.* 52:589-591 (1974).
- Li, et al., "Novel Multifunctional Polymers from Aromatic Diamines by Oxidative Polymerizations," *Chemical Reviews*, vol. 102(9): pp. 2925-2943 (2002).
- Maki, M., et al., "Weather-Resistant Colored Polypropylene," *Chemical Abstracts Service*, ZCPLUS, document No. 89:111364 (1978).
- March, J., *Advanced Organic Chemistry*, McGraw Hill Book Company, New York, pp. 251-259 (1977).
- Masada, H. and Oishi, Y., "A New Synthesis of aryl t-butyl Ethers," *Chem. Letters*, 57-58 (1978).
- Masada, H. et al., "A New Heterogeneous Williamson Synthesis of Ethers Using t-alkyl Substrates," *The Chemical Society of Japan* 3:275-282 (1996).
- Masada, H. et al., "A New Method for the Williamson Ether Synthesis Using t-alkyl Halides in Nonpolar Solvents," *The Chemical Society of Japan*, 2:164-166 (1995).
- Mehdipour-Ataei, S., et al., "Novel Diols Containing Ester and Amide Groups and Resulting Poly(ester amide ester)s," *J. Applied Polymer Sci.*, 93:2699-2703 (2004), XP002420014.
- Mejias, L., et al., "New Polymers From Natural Phenols Using Horse-radish or Soybean Peroxidase," *Macromol. Biosci.*, 2:24-32 (2002).
- Ol'dekop, Yu. A., et al. "Simple Synthesis of the tert-butyl Ether of Phenol" *Inst. Fiz.-Org. Khim., Minsk, USSR. Zhurnal Obshchey Khimii*, 50(2):475-6 (1980).
- Overgaag, M., et al., "Rearrangement of Alkyl Phenyl Ethers Over Dealuminated HY Zeolites Under Liquid-Phase Conditions," *Applied Catalysis A: General*, *Elsevier Sci.*, 175(1-2):139-146 (1998).
- Pátopršty, V., et al., "<sup>13</sup>C NMR Study of 3,9-Di(alkylphenoxy)-2,4,8,10-tetraoxa-3,9-diphosphaspiro[5.5]undecanes," *Magnetic Resonance in Chem.*, 23(2):122-126 (1985).
- PCT Application No. PCT/US2005/001946: International Preliminary Report on Patentability issued Jul. 24, 2006.
- PCT Application No. PCT/US2005/025513: International Preliminary Report on Patentability and Written Opinion mailed on Jan. 23, 2007.
- PCT Application No. PCT/US2005/025646: International Preliminary Report on Patentability mailed on Dec. 20, 2006.
- PCT Application No. PCT/US2005/025646: Written Opinion mailed on Nov. 14, 2006.
- PCT Application No. PCT/US2006/042251: Notification Concerning Transmittal of International Preliminary Report on Patentability mailed on May 8, 2008.
- PCT Application No. PCT/US2006/042251: Notification Concerning Transmittal of International Search Report and Written Opinion of the International Searching Authority, or the Declaration mailed on Feb. 22, 2007.
- PCT Application No. PCT/US2007/015177: Notification Concerning Transmittal of International Preliminary Report on Patentability mailed on Jan. 15, 2009.
- PCT Application No. PCT/US2007/015177: Notification of Transmittal of the International Search Report and Written Opinion of the International Searching Authority, or the Declaration, mailed on Jun. 13, 2008.
- Pirozhenko, V.V., et al., "NMR Study of Topomerization of N-Aroyl-p-Benzoquinonemonoimines," *Russian J. of Organic Chem.*, 31(11):1514-1519 (1995).

(56)

**References Cited**

## OTHER PUBLICATIONS

- Quaschning, V., et al., "Properties of Modified Zirconia Used as Friedel-Crafts-Acylation Catalysts," *J. Catal.* 177:164-174 (1998). RN 85650-63-1, 1984.
- Ryu, K., et al., "Peroxidase-Catalyzed Polymerization of Phenols," *Biocatalysis in Agricultural Biotechnology*, Chapter10:141-157 (1988).
- Sakthivel, A., et al., "Vapour Phase Tertiary Butylation of Phenol Over Sulfated Zirconia Catalyst," *Catal. Lett.*, 72(3-4):225-228 (2001).
- Sartori G., et al., "Highly Selective Mono-tert-butylation of Aromatic Compounds," *Chem. Ind.*, (London), (22):762-763 (1985).
- Scharpe, S.L., et al., "Serine Peptidase Modulators, Their Preparation, and Their Therapeutic Use," Chemical Abstracts Service, ZCPLUS, document No. 131:223514 (1999).

Search Report in international application PCT/US2006/042251 (Feb. 2007).

Singh, A. and Kaplan, D. L., "Biocatalytic Route to Ascorbic Acid-Modified Polymers for Free-Radical Scavenging," *Adv. Matter.*, 15(15):1291-1294 (2003).

Spano, R., et al., "Substituted Anilides of 3-Monoethyl Ester of 4 Hydroxyisophthalic Acid," *J. of Med. Chem.*, 15(5):552-553 (1972).

Thompson, C. Ray, "Stability of Carotene in Alfalfa Meal: Effect of Antioxidants," *Industrial & Engineering Chemistry*, 24(5): 922-925 (1950).

Tsvetkov, O.N., et al., "Alkylation of Phenols with Higher Olefins. Part I," *Int. Chem. Eng.* 7(1):104-121 (1967).

XP-002419239, "Discover Our World of Effects for Polyolefins," *Ciba Speciality Chemicals*, (2003).

Irgafos © 126, BASF publication, pp. 1-3, Jul. 2010.

USPTO Search Report for U.S. Appl. No. 13/572,884, Mar. 20, 2013.

\* cited by examiner

**1**  
**LUBRICANT OIL COMPOSITIONS**

RELATED APPLICATIONS

This application is a continuation of U.S. application Ser. No. 13/165,372, filed Jun. 21, 2011 now abandoned, which is a continuation of U.S. application Ser. No. 11/606,785, filed Nov. 30, 2006 now abandoned, which claims the benefit of U.S. Provisional Application No. 60/742,150, filed on Dec. 2, 2005. The entire teachings of the above applications are incorporated herein by reference.

BACKGROUND OF THE INVENTION

Early lubrication began with animal fats and oils and slowly evolved to petroleum-based oils. Petroleum-based oil, however, do not perform as well as many of the animal-based products and require a lot of refining and treatment. Synthetic oils, which are made from small molecules, have historically had superior lubricating performance characteristics that could not be achieved with conventional oils. However, while many lubricants currently exist, there is still a need for lubricants with improved properties.

SUMMARY OF THE INVENTION

The present invention relates to compositions comprising i) a first antioxidant and at least one first additive, selected from the group comprising surface additives, performance enhancing additives and lubricant protective additives and optionally ii) a second additive and/or a second antioxidant (or stabilizer). These compositions are useful in the methods of the present invention to improve, for example, increase the shelf life, improve the quality and/or performance of lubricants, such as lubricant oils.

In one embodiment, the present invention is a composition comprising a first antioxidant, and at least one first additive selected from the group consisting of i) a surface additive; ii) a performance enhancing additive; and iii) a lubricant protective additive.

In another embodiment the present invention is a lubricant composition comprising: a lubricant or a mixture of lubricants, a first antioxidant and at least one first additive selected from the group consisting of i) a surface additive; ii) a performance enhancing additive; and iii) a lubricant protective additive.

In yet another embodiment the present invention is a method of improving a composition comprising combining the composition with a first antioxidant; and at least one first additive selected from the group consisting of i) a surface additive; ii) a performance enhancing additive; and iii) a lubricant protective additive.

In yet another embodiment the present invention is a method of improving a lubricant or a mixture of lubricants comprising combining the lubricant or mixture of lubricants with a first antioxidant; and at least one first additive selected from the group consisting of i) a surface additive; ii) a performance enhancing additive; and iii) a lubricant protective additive.

The compositions and methods of the present invention generally provide increased shelf life, increased oxidative resistance, enhanced performance and/or improved quality to materials, such as, for example, lubricants and lubricant oils. In general it is believed that because of the synergy of the antioxidants with the additives, the compositions described herein have superior oxidation resistance. The additives exhibit several key functions such as corrosion inhibition, detergency, viscosity modification, antiwear performance, dispersant properties, cleaning and suspending ability. The disclosed compositions, in general provide superior perfor-

mance of lubricants in high temperatures applications due to the presence of antioxidants which are thermally stable at high temperatures with enhanced oxidation resistance.

5      DETAILED DESCRIPTION OF THE INVENTION

The present invention relates to compositions for improving lubricants, wherein the compositions comprise i) a first antioxidant selected from the group comprising of antioxidants described in Provisional Patent Application Nos. 60/632,893, 60/633,197, 60/633,252, 60/633,196, 60/665, 638, 60/655,169, 60/731,125, 60/731,021 and 60/731,325; U.S. patent application Ser. Nos. 11/184,724, 11/184,716, 11/040,193, 10/761,933, 10/408,679 and 10/761,933; PCT Patent Application Nos. PCT/US2005/001948, PCT/US2005/001946 and PCT/US03/10782, the entire contents of each of which are incorporated herein by reference; along with at least one first additive selected from the groups comprising of surface additives, performance enhancing additives and lubricant protective additives; and optionally ii) a second additive and/or a second antioxidant (or stabilizer) wherein examples of suitable second additives and antioxidants are as described herein.

In one embodiment, the first antioxidants which are suitable for use in the compositions and methods of the present invention include, but are not limited to: polyalkyl phenol based antioxidants, sterically hindered phenol based antioxidants, sterically hindered phenol based macromolecular antioxidants, nitrogen and hindered phenol containing dual functional macromolecular antioxidants, alkylated macromolecular antioxidants, sterically hindered phenol and phosphite based macromolecular antioxidants.

In one embodiment, the first antioxidants which are suitable for use in the compositions and methods of the present invention include antioxidant polymers which comprises repeat units that include one or both of Structural Formulas (I) and (II):



where:

R is —H or a substituted or unsubstituted alkyl, substituted or unsubstituted acyl or substituted or unsubstituted aryl group;

Ring A is substituted with at least one tert-butyl group or substituted or unsubstituted n-alkoxycarbonyl group, and optionally one or more groups selected from the group consisting of —OH, —NH, —SH, a substituted or unsubstituted alkyl or aryl group, and a substituted or unsubstituted alkoxy carbonyl group;

Ring B is substituted with at least one —H and at least one tert-butyl group or substituted or unsubstituted n-alkoxycarbonyl group and optionally one or more groups selected from the group consisting of —OH,

3

—NH, —SH, a substituted or unsubstituted alkyl or aryl group, and a substituted or unsubstituted alkoxy carbonyl group;

n is an integer equal to or greater than 2; and

p is an integer equal to or greater than 0.

In another embodiment, the first antioxidants which are suitable for use in the compositions and methods of the present invention include polymers with repeat units represented by one or both of Structural Formulas (III) and (IV):



(III)



(IV)

where Rings A and B are substituted as described above and n and p are as defined above.

Preferably, Ring A and Ring B in Structural Formulas (I) to (IV) are each substituted with at least one tert-butyl group.

In another embodiment, the first antioxidants which are suitable for use in the compositions and methods of the present invention include polymers with repeat units represented by one or more of Structural Formulas (Va), (Vb), (Vc), (VIa), (VIb) and (VIc):



(Va)



(Vb)



(Vc)

4

-continued

(VIa)



(VIb)



(VIc)



where  $R_1$ ,  $R_2$  and  $R_3$  are independently selected from the group consisting of —H, —OH, —NH, —SH, a substituted or unsubstituted alkyl or a substituted or unsubstituted aryl group, and a substituted or unsubstituted alkoxy carbonyl group, provided that at least one of  $R_1$ ,  $R_2$  and  $R_3$  is a tert-butyl group; and  $j$  and  $k$  are independently integers of zero or greater, such that the sum of  $j$  and  $k$  is equal to or greater than 2.

In a particular embodiment,  $R$  is —H or —CH<sub>3</sub>;  $R_2$  is —H, —OH, or a substituted or unsubstituted alkyl group; or both.

Specific examples of repeat units included in polymers which are suitable for use in the compositions and methods of the present invention are represented by one of the following structural formulas:



(VII)



(VIII)

5  
-continued6  
-continued

Antioxidant polymers as described immediately above which are suitable for use in the compositions and methods of the present invention have two or more repeat units, preferably greater than about five repeat units. The molecular weight of the polymers disclosed above is generally selected to be appropriate for the desired application. Typically, the molecular weight is greater than about 500 atomic mass units (amu) and less than about 2,000,000 amu, greater than about 1000 amu and less than about 100,000, greater than about 2,000 amu and less than about 10,000, or greater than about 2,000 amu and less than about 5,000 amu.

Antioxidant polymers as described immediately above which are suitable for use in the compositions and methods of the present invention can be either homopolymers or copolymers. A copolymer preferably contains two or more or three or more different repeating monomer units, each of which has varying or identical antioxidant properties. The identity of the repeat units in a copolymer can be chosen to modify the antioxidant properties of the polymer as a whole, thereby giving a polymer with tunable properties. The second, third and/or further repeat units in a copolymer can be either a synthetic or natural antioxidant.

Antioxidant polymers as described immediately above which are suitable for use in the compositions and methods of the present invention are typically insoluble in aqueous media. The solubility of the antioxidant polymers in non-aqueous media (e.g., oils) depends upon the molecular weight of the polymer, such that high molecular weight polymers are typically sparingly soluble in non-aqueous media. When an antioxidant polymer of the invention is insoluble in a particular medium or substrate, it is preferably well-mixed with that medium or substrate.

Antioxidant polymers as described immediately above which are suitable for use in the compositions and methods of the present invention can be branched or linear, but are preferably linear. Branched antioxidant polymers can only be

formed from benzene molecules having three or fewer substituents (e.g., three or more hydrogen atoms), as in Structural Formulas (XX), (XXI) and (XXIV).

In another embodiment, the first antioxidants which are suitable for use in the compositions and methods of the present invention include polymers with repeat units represented by one or both of Structural Formulas (I) and (II):



where:

R is —H or a substituted or unsubstituted alkyl, acyl or aryl group;

Ring A is substituted with at least one tert-butyl group, 1-ethenyl-2-carboxylic acid group or ester thereof, substituted or unsubstituted alkyleneoxy group, or substituted or unsubstituted n-alkoxycarbonyl group and zero, one or more additional functional groups;

Ring B is substituted with at least one —H and at least one tert-butyl group, 1-ethenyl-2-carboxylic acid group or ester thereof, substituted or unsubstituted alkyleneoxy group, or substituted or unsubstituted n-alkoxycarbonyl group and zero, one or more additional functional groups;

n is an integer equal to or greater than 2; and

p is an integer equal to or greater than 0,

where the polymer includes two or more repeat units represented by one or both of Structural Formulas (I) and (II) that are directly connected by a C—C or C—O—C bond between benzene rings.

Polymers as described immediately above which are suitable for use in the compositions and methods of the present invention that do not include any repeat units represented by Structural Formula (I) are preferably substituted on Ring B with one or more hydroxyl or acyloxy groups.

Repeat units of the antioxidant polymers as described immediately above which are suitable for use in the compositions and methods of the present invention include substituted benzene molecules. These benzene molecules are typically based on phenol or a phenol derivative, such that they have at least one hydroxyl, ester or ether functional group. Preferably, the benzene molecules have a hydroxyl group. The hydroxyl group is not restricted to being a free hydroxyl group, and the hydroxyl group can be protected or have a cleavable group attached to it (e.g., an ester group). Such cleavable groups can be released under certain conditions (e.g., changes in pH), with a desired shelf life or with a time-controlled release (e.g., measured by the half-life), which allows one to control where and/or when an antioxidant polymer is able to exert its antioxidant effect.

Substituted benzene repeat units of an antioxidant polymer as described immediately above which are suitable for use in the compositions and methods of the present invention are also typically substituted with a bulky alkyl group, a 1-ethenyl-2-carboxylic acid group, a substituted or unsubstituted alkyleneoxy group, or an n-alkoxycarbonyl group. Prefer-

ably, the benzene monomers are substituted with a bulky alkyl group. More preferably, the bulky alkyl group is located ortho or meta to a hydroxyl group on the benzene ring. A “bulky alkyl group” is defined herein as an alkyl group that is branched alpha- or beta- to the benzene ring. Preferably, the alkyl group is branched alpha to the benzene ring. More preferably, the alkyl group is branched twice alpha to the benzene ring (i.e., to form an alpha-tertiary carbon), such as in a tert-butyl group. Other examples of bulky alkyl groups include isopropyl, 2-butyl, 3-pentyl, 1,1-dimethylpropyl, 1-ethyl-1-methylpropyl and 1,1-diethylpropyl. The bulky alkyl groups are preferably unsubstituted, but they can be substituted with a functional group that does not interfere with the antioxidant activity of the molecule or the polymer.

Substituted benzene repeat units that are substituted with a substituted or unsubstituted alkyleneoxy group typically have an unsubstituted alkyleneoxy group. Substituted alkyleneoxy groups are also suitable, although the substituents should not interfere with the antioxidant activity of the molecule or the polymer. Typically, an alkyleneoxy group is a lower alkyleneoxy group, such as a methyleneoxy group or an ethyleneoxy group. A methyleneoxy group is preferred (as in sesamol).

Straight chained alkoxycarbonyl groups typically have an alkyl chain of one to sixteen carbon atoms, and include methoxycarbonyl, ethoxycarbonyl, n-propoxycarbonyl, n-butoxycarbonyl and n-pentoxycarbonyl. n-propoxycarbonyl is a preferred group. Similar to the bulky alkyl groups, n-alkoxycarbonyl groups are optionally substituted with a functional group that does not interfere with the antioxidant activity of the molecule or the polymer. Alkoxycarbonyl groups can also be present in their hydrolyzed form, namely as carboxy groups or carboxylic acid groups.

In substituted benzene repeat units having a 1-ethenyl-2-carboxylic acid group or an ester thereof, the 1-carbon (i.e., the carbon distal from the carboxylic acid moiety) is attached to the benzene ring.

In addition to the substituents named above, substituted benzene repeat units can have additional functional groups as substituents. For example, the additional functional groups can be selected from the group consisting of —OH, —NH, —SH, a substituted or unsubstituted alkyl or aryl group, a substituted or unsubstituted alkoxycarbonyl group, a substituted or unsubstituted alkoxy group and a saturated or unsaturated carboxylic acid group. Typically, the additional functional groups are selected from the group consisting of —OH, a substituted or unsubstituted alkoxy group and a saturated or unsaturated carboxylic acid group.

Preferably, Ring A and Ring B in Structural Formulas (I) to (IV) are each substituted with at least one tert-butyl group.

Further, specific examples of repeat units included in polymers which are suitable for use in the compositions and methods of the present invention are represented by one of the following structural formulas:

(XVIIIa)



-continued



(XVIIIb)

(XVIIIc)

Antioxidant polymers as described immediately above which are suitable for use in the methods and compositions of the present invention are typically insoluble in aqueous media, although certain polymers of gallic acid and its esters are water soluble. The solubility of the antioxidant polymers in non-aqueous media (e.g., oils) depends upon the molecular weight of the polymer, such that high molecular weight polymers are typically sparingly soluble in non-aqueous media. When an antioxidant polymer of the invention is insoluble in a particular medium or substrate, it is preferably well-mixed with that medium or substrate.

Antioxidant polymers as described immediately above which are suitable for use in the methods and compositions of the present invention can be branched or linear, but are preferably linear. Branched antioxidant polymers can only be formed from benzene molecules having three or fewer substituents (e.g., three or more hydrogen atoms), as in Structural Formulas (XX), (XXI) and (XXIV).

In another embodiment, the first antioxidants which are suitable for use in the compositions and methods of the present invention include a polyalkylphenol antioxidant represented by Structural Formula U or U'.

Although Structural Formulas (XI), (XVI), (XVII) and (XVIII) are represented as having a propoxycarbonyl substituent, this group can generally be replaced with a different C<sub>1</sub>-C<sub>16</sub> n-alkoxycarbonyl group or can be a carboxylate group.

A particular polymer suitable for use in the methods and compositions of the present invention is poly(2-tert-butyl-4-hydroxyanisole).

Antioxidant polymers as described immediately above which are suitable for use in the methods and compositions of the present invention have two or more repeat units, preferably greater than about five repeat units. The molecular weight of the polymers disclosed herein is generally selected to be appropriate for the desired application. Typically, the molecular weight is greater than about 500 atomic mass units (amu) and less than about 2,000,000 amu, greater than about 1000 amu and less than about 100,000, greater than about 2,000 amu and less than about 10,000 amu, or greater than about 2,000 amu and less than about 5,000 amu.

Antioxidant polymers as described immediately above which are suitable for use in the methods and compositions of the present invention can be either homopolymers or copolymers. A copolymer preferably contains two or more or three or more different repeating monomer units, each of which has varying or identical antioxidant properties (including monomers having no antioxidant activity). The identity of the repeat units in a copolymer can be chosen to modify the antioxidant properties of the polymer as a whole, thereby giving a polymer with tunable properties. The second, third and/or further repeat units in a copolymer can be either a synthetic or natural antioxidant. In one example, a composition of the invention includes one or more homopolymers and one or more copolymers (e.g., in a blend). Preferably, both homopolymers and copolymers include two or more substituted benzene repeat units that are directly connected by a C—C or C—O—C bond. Preferably, at least 50%, such as at least 70%, for example, at least 80%, but preferably about 100% of the repeat units in a copolymer are substituted benzene repeat units directly connected by a C—C or C—O—C bond.

Examples of copolymers include poly(TBHQ-co-propyl gallate), poly(TBHQ-co-BHA), poly(TBHQ-co-sesamol), poly(BHA-co-sesamol), poly(propyl gallate-co-sesamol) and poly(BHA-co-propyl gallate). The ratio of one monomer to another, on a molar basis, is typically about 100:1 to about 1:100, such as about 10:1 to about 1:10, for example, about 2:1 to about 1:2. In one example, the ratio of monomers is about 1:1.

20 In another embodiment, the first antioxidants which are suitable for use in the compositions and methods of the present invention include a polyalkylphenol antioxidant represented by Structural Formula U or U'.



U  
In Structural Formula U or U', n is an integer equal or greater than 2. R is a C<sub>1</sub>-C<sub>10</sub> alkyl group, an aryl group, or a benzyl group. Typically, R is a tertiary alkyl group, or in preferred embodiments, a tertiary butyl group. X is —O—, —NH— or —S—. Each R<sub>10</sub> is independently an optionally substituted C<sub>1</sub>-C<sub>10</sub> alkyl group, an optionally substituted aryl group, and optionally substituted alkoxy group, an optionally substituted carbonyl group, an optionally substituted alkoxy carbonyl group, —OH, —SH or —NH<sub>2</sub>; or two R<sub>10</sub> groups on adjacent carbon atoms join together to form an optionally substituted aromatic ring or an optionally substituted carbocyclic or heterocyclic non-aromatic ring. q is an integer from 0 to 2.

U'  
Repeat units of the antioxidant polymers as described immediately above which are suitable for use in the compositions and methods of the present invention include substituted benzene molecules. These benzene molecules are typically based on phenol or a phenol derivative, such that they have at least one hydroxyl or ether functional group. Preferably, the benzene molecules have a hydroxyl group. The hydroxyl group can be a free hydroxyl group and can be protected or have a cleavable group attached to it (e.g., an ester group). Such cleavable groups can be released under certain conditions (e.g., changes in pH), with a desired shelf

## 11

life or with a time-controlled release (e.g., measured by the half-life), which allows one to control where and/or when an antioxidant polymer can exert its antioxidant effect. The repeat units can also include analogous thiophenol and aniline derivatives, e.g., where the phenol —OH can be replaced by —SH, —NH—, and the like.

Substituted benzene repeat units of an antioxidant polymer as described immediately above which are suitable for use in the compositions and methods of the present invention are also typically substituted with a bulky alkyl group or an n-alkoxycarbonyl group. Preferably, the benzene monomers are substituted with a bulky alkyl group. More preferably, the bulky alkyl group is located ortho or meta to a hydroxyl group on the benzene ring, typically ortho. A “bulky alkyl group” is defined herein as an alkyl group that is branched alpha- or beta- to the benzene ring. Preferably, the alkyl group is branched alpha to the benzene ring. More preferably, the alkyl group is branched twice alpha to the benzene ring, such as in a tert-butyl group. Other examples of bulky alkyl groups include isopropyl, 2-butyl, 3-pentyl, 1,1-dimethylpropyl, 1-ethyl-1-methylpropyl and 1,1-diethylpropyl. The bulky alkyl groups are preferably unsubstituted, but they can be substituted with a functional group that does not interfere with the antioxidant activity of the molecule or the polymer. Straight chained alkoxy carbonyl groups include methoxy carbonyl, ethoxycarbonyl, n-propoxycarbonyl, n-butoxycarbonyl and n-pentoxycarbonyl. n-propoxycarbonyl is a preferred group. Similar to the bulky alkyl groups, n-alkoxycarbonyl groups are optionally substituted with a functional group that does not interfere with the antioxidant activity of the molecule or the polymer.

In another embodiment, the first antioxidants which are suitable for use in the compositions and methods of the present invention include a polymer comprising repeat units represented by one or both of Structural Formulas (i) and (ii):



where:

Ring A is substituted with at least one tert-butyl group, and optionally one or more groups selected from the group consisting of a substituted or unsubstituted alkyl or aryl group, and a substituted or unsubstituted alkoxy carbonyl group;

Ring B is substituted with at least one —H and at least one tert-butyl group and optionally one or more groups selected from the group consisting of—a substituted or unsubstituted alkyl or aryl group, and a substituted or unsubstituted alkoxy carbonyl group;

n is an integer equal to or greater than 2; and  
p is an integer equal to or greater than 0.

## 12

In another embodiment, the first antioxidants which are suitable for use in the compositions and methods of the present invention are polymers represented by one or both of Structural Formulas (iv) and (v):



where Ring A is substituted with at least one tert-butyl group, and optionally one or more groups selected from the group consisting of a substituted or unsubstituted alkyl or aryl group, and a substituted or unsubstituted alkoxy carbonyl group; Ring B is substituted with at least one —H and at least one tert-butyl group and optionally one or more groups selected from the group consisting of a substituted or unsubstituted alkyl or aryl group, and a substituted or unsubstituted alkoxy carbonyl group; R is —H, an optionally substituted C1-C10 alkyl group, an aryl group, a benzyl group, or an acyl group n is an integer equal to or greater than 2; and p is an integer equal to or greater than 0. In one embodiment R is a C1-10 branched or linear alkyl group.

Antioxidant polymers as described immediately above which are suitable for use in the methods of the present invention have two or more repeat units, preferably greater than about five repeat units. The molecular weight of the polymers disclosed herein can be generally selected to be appropriate for the desired application. Typically, the molecular weight can be greater than about 500 atomic mass units (amu) and less than about 2,000,000 amu, greater than about 1,000 amu and less than about 100,000, greater than about 2,000 amu and less than about 10,000, or greater than about 2,000 amu and less than about 5,000 amu.

Antioxidant polymers as described immediately above which are suitable for use in the methods of the present invention can be either homopolymers or copolymers. A copolymer preferably contains two or more or three or more different repeating monomer units, each of which has varying or identical antioxidant properties. The identity of the repeat units in a copolymer can be chosen to modify the antioxidant properties of the polymer as a whole, thereby giving a polymer with tunable properties. The second, third and/or further repeat units in a copolymer can be either a synthetic or natural antioxidant.

Antioxidant polymers as described immediately above which are suitable for use in the methods of the present invention are typically insoluble in aqueous media. The solubility of the antioxidant polymers in non-aqueous media (e.g., oils) depends upon the molecular weight of the polymer, such that high molecular weight polymers are typically sparingly soluble in non-aqueous media. When an antioxidant polymer of the invention can be insoluble in a particular medium or substrate, it can be preferably well-mixed with that medium or substrate.

## 13

Antioxidant polymers as described immediately above which are suitable for use in the methods of the present invention can be branched or linear, but are preferably linear. Branched antioxidant polymers can only be formed from benzene molecules having three or fewer substituents (e.g., three or more hydrogen atoms), as in Structural Formulas (XX), (XXI) and (XXIV).

Another specific example of a repeat unit included in polymers which are suitable for use in the compositions and methods of the present invention is represented by the following structural formula:



In another embodiment, the first antioxidant polymers which are suitable for use in the compositions and methods of the present invention includes a macromolecule which can be represented by one or both of Structural Formulas R and S:



In Structural Formulas R and S, n is an integer equal to or greater than 2.

The variable X is O, NH, or S.

The variable Z is H.

Each variable K is independently —H or —OH, with at least one —OH adjacent to a —H; or K is a bond when that position is involved in the polymer chain.

In another embodiment, the first antioxidants which are suitable for use in the compositions and methods of the present invention includes a macromolecular antioxidant polymer represented by one or both of Structural Formulas T and V or T' and V':



## 14

-continued

V



T'



V'



25

R In Structural Formulas T, T', V and V', n is an integer equal to or greater than 2.

The variable X is O, NH, or S.

The variable Z is H.

Each variable R is independently —H, —OH, a C1-C10 alkyl group, or a bond when that position is involved in the polymer chain wherein at least one —OH is adjacent to a C1-C10 alkyl group, e.g., a tertiary butyl group.

Each R<sub>10</sub> is independently an optionally substituted C1-C10 alkyl group, an optionally substituted aryl group, and optionally substituted alkoxy group, an optionally substituted carbonyl group, an optionally substituted alkoxy carbonyl group, an optionally substituted aryloxy carbonyl group, —OH, —SH or —NH<sub>2</sub> or two R<sub>10</sub> groups on adjacent carbon atoms join together to form an optionally substituted aromatic ring or an optionally substituted carbocyclic or heterocyclic non-aromatic ring. q is an integer from 0 to 2. R<sub>12</sub> is a bulky alkyl group substituent bonded to a ring carbon atom adjacent (ortho) to a ring carbon atom substituted with an —OH group.

n is an integer equal to or greater than 2.

These macromolecular antioxidant polymers can contain, for example, tert-butylhydroquinone, 2,5-di-tert-butylhydroquinone, BHT type repeat units and their combinations. In some embodiments, of the macromolecular antioxidants described immediately above can be homopolymers, copolymers, terpolymers, and the like.

Substituted benzene repeat units of an antioxidant polymer as described immediately above which are suitable for use in the methods and compositions of the present invention are typically substituted with a bulky alkyl group or an n-alkoxy carbonyl group. Preferably, the benzene monomers are substituted with a bulky alkyl group. More preferably, the bulky alkyl group is located ortho or meta to a hydroxyl group on the benzene ring, typically ortho. A "bulky alkyl group" is defined herein as an alkyl group that is branched alpha- or beta- to the benzene ring. Preferably, the alkyl group is branched alpha to the benzene ring. More preferably, the alkyl group is branched twice alpha to the benzene ring, such as in a tert-butyl group. Other examples of bulky alkyl groups include isopropyl, 2-butyl, 3-pentyl, 1,1-dimethylpropyl, 1-ethyl-1-methylpropyl and 1,1-diethylpropyl. The bulky alkyl groups are preferably unsubstituted, but they can be

T

55

60

65

substituted with a functional group that does not interfere with the antioxidant activity of the molecule or the polymer. Straight chained alkoxy carbonyl groups include methoxy carbonyl, ethoxycarbonyl, n-propoxycarbonyl, n-butoxycarbonyl and n-pentoxy carbonyl. n-propoxycarbonyl is a preferred group. Similar to the bulky alkyl groups, n-alkoxycarbonyl groups are optionally substituted with a functional group that does not interfere with the antioxidant activity of the molecule or the polymer.

Antioxidant polymers as described immediately above which are suitable for use in the methods and compositions of the present invention have two or more repeat units, preferably greater than about five repeat units. The molecular weight of the polymers disclosed herein can be generally selected to be appropriate for the desired application. Typically, the molecular weight can be greater than about 500 atomic mass units (amu) and less than about 2,000,000 amu, greater than about 1,000 amu and less than about 100,000, greater than about 2,000 amu and less than about 10,000, or greater than about 2,000 amu and less than about 5,000 amu.

Antioxidant polymers as described immediately above which are suitable for use in the methods and compositions of the present invention can be either homopolymers or copolymers. A copolymer preferably contains two or more or three or more different repeating monomer units, each of which has varying or identical antioxidant properties. The identity of the

repeat units in a copolymer can be chosen to modify the antioxidant properties of the polymer as a whole, thereby giving a polymer with tunable properties. The second, third and/or further repeat units in a copolymer can be either a synthetic or natural antioxidant.

Antioxidant polymers as described immediately above which are suitable for use in the methods and compositions of the present invention are typically insoluble in aqueous media. The solubility of the antioxidant polymers in non-aqueous media (e.g., oils) depends upon the molecular weight of the polymer, such that high molecular weight polymers are typically sparingly soluble in non-aqueous media. When an antioxidant polymer of the invention can be insoluble in a particular medium or substrate, it can be preferably well-mixed with that medium or substrate.

Antioxidant polymers as described immediately above which are suitable for use in the methods and compositions of the present invention can be branched or linear, but are preferably linear. Branched antioxidant polymers can only be formed from benzene molecules having three or fewer substituents (e.g., three or more hydrogen atoms), as in Structural Formulas (XX), (XXI) and (XXIV).

Specific examples of repeat units included in polymers which are suitable for use in the compositions and methods of the present invention are represented by one of the following structural formulas:



-continued



n is an integer equal to or greater than 2.

In another embodiment, the first antioxidants which are suitable for use in the compositions and methods of the present invention includes an antioxidant polymer represented by Structural Formula M or M'.



In Structural Formula M:  
n is an integer equal to or greater than 2;  
R<sub>1</sub> is O, S, or NH;

40 R<sub>4</sub>, R<sub>5</sub>, R<sub>7</sub> and R<sub>8</sub> are independently —H, —OH, —NH,  
—SH, a substituted or unsubstituted alkyl or aryl group,  
or a substituted or unsubstituted alkoxy carbonyl group,  
or a bond when part of the polymer chain,  
provided that:

45 (1) at least one of R<sub>4</sub>, R<sub>5</sub>, R<sub>7</sub> and R<sub>8</sub> is a tert-butyl group or  
a substituted or unsubstituted alkoxy carbonyl group, and at  
least two of R<sub>4</sub>, R<sub>5</sub>, R<sub>7</sub> and R<sub>8</sub> are —H; or

50 (2) at least one of R<sub>4</sub>, R<sub>5</sub>, R<sub>7</sub> and R<sub>8</sub> is a tert-butyl group or  
a substituted or unsubstituted alkoxy carbonyl group, at least  
one of R<sub>4</sub>, R<sub>5</sub>, R<sub>7</sub> and R<sub>8</sub> is a hydroxyl, alkoxy, alkoxy carbonyl  
or aryloxy carbonyl group, and at least one of R<sub>4</sub>, R<sub>5</sub>, R<sub>7</sub>  
and R<sub>8</sub> is —H.

55 In structural formula M' each X is independently —O—,  
—NH— or —S—. Each R<sub>10</sub> is independently an optionally  
substituted C1-C10 alkyl group, an optionally substituted  
aryl group, and optionally substituted alkoxy group, an  
optionally substituted carbonyl group, an optionally substituted  
alkoxy carbonyl group, an optionally substituted aryloxy carbonyl  
group, —OH, —SH or —NH<sub>2</sub>; and/or two R<sub>10</sub>  
groups on adjacent carbon atoms join together to form an  
optionally substituted aromatic ring or an optionally substituted  
carbocyclic or heterocyclic non-aromatic ring. q is an  
integer from 0 to 2. n is an integer greater than or equal to 2.

60 65 Substituted benzene repeat units of an antioxidant polymer  
as described immediately above which are suitable for use in  
the methods and compositions of the present invention are

also typically substituted with a bulky alkyl group or an n-alkoxycarbonyl group. Preferably, the benzene monomers are substituted with a bulky alkyl group. More preferably, the bulky alkyl group is located ortho or meta to a hydroxyl group on the benzene ring, typically ortho. A “bulky alkyl group” is defined herein as an alkyl group that is branched alpha- or beta- to the benzene ring. Preferably, the alkyl group is branched alpha to the benzene ring. More preferably, the alkyl group is branched twice alpha to the benzene ring, such as in a tert-butyl group. Other examples of bulky alkyl groups include isopropyl, 2-butyl, 3-pentyl, 1,1-dimethylpropyl, 1-ethyl-1-methylpropyl and 1,1-diethylpropyl. The bulky alkyl groups are preferably unsubstituted, but they can be substituted with a functional group that does not interfere with the antioxidant activity of the molecule or the polymer. Straight chained alkoxy carbonyl groups include methoxy carbonyl, ethoxycarbonyl, n-propoxycarbonyl, n-butoxycarbonyl and n-pentoxycarbonyl. n-propoxycarbonyl is a preferred group. Similar to the bulky alkyl groups, n-alkoxycarbonyl groups are optionally substituted with a functional group that does not interfere with the antioxidant activity of the molecule or the polymer.

Antioxidant polymers as described immediately above which are suitable for use in the methods and compositions of the present invention have two or more repeat units, preferably greater than about five repeat units. The molecular weight of the polymers disclosed herein can be generally selected to be appropriate for the desired application. Typically, the molecular weight can be greater than about 500 atomic mass units (amu) and less than about 2,000,000 amu, greater than about 1,000 amu and less than about 100,000, greater than about 2,000 amu and less than about 10,000, or greater than about 2,000 amu and less than about 5,000 amu.

Antioxidant polymers as described immediately above which are suitable for use in the methods and compositions of the present invention can be either homopolymers or copolymers. A copolymer preferably contains two or more or three or more different repeating monomer units, each of which has varying or identical antioxidant properties. The identity of the repeat units in a copolymer can be chosen to modify the antioxidant properties of the polymer as a whole, thereby giving a polymer with tunable properties. The second, third and/or further repeat units in a copolymer can be either a synthetic or natural antioxidant.

Antioxidant polymers as described immediately above which are suitable for use in the methods and compositions of the present invention are typically insoluble in aqueous media. The solubility of the antioxidant polymers in non-aqueous media (e.g., oils) depends upon the molecular weight of the polymer, such that high molecular weight polymers are typically sparingly soluble in non-aqueous media. When an antioxidant polymer of the invention can be insoluble in a particular medium or substrate, it can be preferably well-mixed with that medium or substrate.

Antioxidant polymers as described immediately above which are suitable for use in the methods and compositions of the present invention can be branched or linear, but are preferably linear. Branched antioxidant polymers can only be formed from benzene molecules having three or fewer substituents (e.g., three or more hydrogen atoms), as in Structural Formulas (XX), (XXI) and (XXIV).

In another embodiment, the first antioxidants which are suitable for use in the compositions and methods of the present invention include a polymer having at least one repeat unit that is represented by a structure selected from the group consisting of Structural Formulas (A), (B), (C), (D) and combinations thereof:



R' is a covalent bond, —O—, —C(O)O—, —C(O)N—, —C(O)—, —CH=CH—, —S— or —N—.

R<sub>1</sub> is —H or an alkyl group, or —(CH<sub>2</sub>)<sub>k</sub>—O—X—Z. Typically, R<sub>1</sub> is —H or alkyl.

Each X is independently a covalent bond, —C(O)—, —C(O)O— or —C(O)N—.

Y is —O—, —N— or —S—.

Each Z is an independently selected antioxidant.

a is an integer from 0 to 12.

Each k is independently an integer from 0 to 12.

m is an integer from 0 to 6.

n is 0 or 1.

p is an integer from 0 to 6.

In one embodiment, the polymer does not include cyclic anhydride repeat units.

An antioxidant can be attached to the polymer by one or more linkages or bonds. Examples of suitable linkages include acetal, amide, amine, carbamate, carbonate, ester, ether and thioether linkage. Carbon-carbon bonds can be also suitable. As used herein, an amide is distinguished from a diacyl hydrazide.

There are many examples of polymers that can be derivatized with an antioxidant. One type of such polymer has pendant hydroxyl groups, such as poly(vinyl alcohol) and copolymers thereof (e.g., poly(ethylene-co-vinyl alcohol)). The hydroxyl groups of poly(vinyl alcohol), a polyhydroxy-alkyl methacrylate (e.g., polyhydroxy methyl methacrylate), and poly(ethylene-co-vinyl alcohol) react with an antioxidant to form the derivatized antioxidant polymer. Another type of derivatizable polymer contains pendant carboxylic acid groups or esters thereof, such as poly(acrylic acid), poly(alkylacrylic acid) and esters thereof. Poly(acrylic acid) is a preferred polymer; the carboxylic acid groups of poly(acrylic acid) can be derivatized, although carboxylic acid groups generally require activation before derivatization can occur.

An additional type of derivatizable polymer can be a poly(substituted phenol), where the substituted phenol has a substituent with a nucleophilic or electrophilic moiety. Such poly(substituted phenols) can include repeat units represented by the following structural formulas:



where  $a$  is an integer from 0 to 12;  $R$  is  $-\text{OH}$ ,  $-\text{COOH}$ ,  $-\text{NH}_2$ ,  $-\text{SH}$  or a halogen; and  $R_{10}$ ,  $R_{11}$  and  $R_{12}$  are each independently  $-\text{H}$ ,  $-\text{OH}$ ,  $-\text{NH}_2$  or  $-\text{SH}$ , provided that at least one of  $R_{10}$ ,  $R_{11}$  and  $R_{12}$  is  $-\text{OH}$ ,  $-\text{NH}_2$  or  $-\text{SH}$ . Preferably, one of  $R_{10}$ ,  $R_{11}$  and  $R_{12}$  is  $-\text{OH}$  and the remaining two are optionally  $-\text{H}$ . More preferably,  $R_{11}$  is  $-\text{OH}$  and  $R_{10}$  and  $R_{12}$  are  $-\text{H}$ .

The derivatizable polymers can be homopolymers or copolymers. Copolymers include, for example, block, star, hyperbranched, random, gradient block, and alternate copolymers. The derivatizable polymers can be branched or linear, but are preferably linear.

In copolymers, it is only necessary for one repeat unit to include a pendant reactive group. Second and further repeat units of a copolymer can optionally include a pendant reactive group. For example, about 1% to 100%, such as 10% to 50% or 50% to 100%, of the repeat units of a polymer include pendant functional groups.

All or a fraction of the pendant reactive groups of a derivatizable polymer can be derivatized with an antioxidant. In one example, about 100% of the pendant reactive groups can be derivatized. In another example, about 5% to about 90%, such as about 20% to about 80% (e.g., about 50% to about 80%) of the pendant reactive groups can be derivatized.

These polymers can be minimally derivatized with a single type of antioxidant, but can be derivatized with two or more antioxidants (e.g., chemically distinct antioxidants). When there can be two or more antioxidants, they can be in the same class, as described below, or can be in different classes. The ratio of antioxidants can be varied in order to obtain a polymer having a desired set of properties. For example, when a polymer can be derivatized with two antioxidants, the ratio of a first antioxidant to a second antioxidant can be from about 20:1 to about 1:20, such as from about 5:1 to about 1:5 (e.g., about 1:1).

Many antioxidants can be suitable, provided that they can be attached to a polymer and retain their antioxidant activity.

One class of suitable antioxidants can be phenolic antioxidants. Phenolic antioxidants typically have one or more bulky alkyl groups (alkyl groups having a secondary or tertiary carbon alpha to the phenol ring) ortho or meta, preferably ortho, to the phenol hydroxyl group. Phenolic antioxidants can alternatively have an alkyleneoxy substituent, an alkoxy carbonyl substituent, a 1-propenyl-3-carboxylic acid substituent or an ester thereof. A preferred bulky alkyl group is a tert-butyl group. The phenol hydroxyl group can be protected by a removable protecting group (e.g., an acyl group). Phenolic antioxidants for use in the present invention also generally have a substituent that can react with the pendant reactive group of one of the polymers described above to form a covalent bond between the antioxidant and the polymer.

One group of suitable phenolic antioxidants can be represented by Structural Formula (E):



$R_9$  is  $-\text{H}$  or a substituted or unsubstituted alkyl, acyl or aryl group, preferably  $-\text{H}$  or an acyl group.

$R_4$ ,  $R_5$ ,  $R_6$ ,  $R_7$  and  $R_8$  are independently chosen substituent groups, such that at least one substituent can be a substituted or unsubstituted alkyl or aryl group, a substituted or unsubstituted alkoxy carbonyl group, a substituted or unsubstituted alkyleneoxy group, a 1-propenyl-3-carboxylic acid group or an ester thereof. Also, at least one of  $R_4$ ,  $R_5$ ,  $R_6$ ,  $R_7$  and  $R_8$  must be a substituent capable of reacting with the pendant reactive group of the polymers described above, such as a substituent having a nucleophilic or electrophilic moiety. Other suitable substituents include, for example,  $-\text{H}$ ,  $-\text{OH}$ ,  $-\text{NH}$  and  $-\text{SH}$ . A substituent should not decrease the antioxidant activity more than two-fold; instead, substituents preferably increase the antioxidant activity of the molecule.

Specific examples of phenolic antioxidants that can be attached to a polymer include phenolic antioxidant can be selected from the group consisting of 3-(3,5-di-tert-butyl-4-hydroxyphenyl) propionic acid, 3,5-di-tert-butyl-4-hydroxybenzenethiol, 2-(3,5-di-tert-butyl-4-hydroxyphenyl)acetic acid, 3,5-di-tert-butyl-4-hydroxybenzoic acid, 3,5-di-tert-butyl-4-hydroxycinnamic acid, gallic acid, alkyl gallates, 3,5-di-tert-butyl-4-hydroxybenzyl alcohol, tert-butyl-hydroquinone, 2,5-di-tert-butyl-hydroquinone, 2,6-di-tert-butyl-hydroquinone, 3,5-di-tert-butyl-4-hydroxybenzaldehyde, monoacetoxy-tert-butylhydroquinone, sesamol, isoflavones, flavonoids and coumarins.

Another antioxidant that can be attached to one of the polymers described immediately above can be ascorbic acid or a molecule that contains an ascorbic acid moiety. Typically, ascorbic acid attached to a polymer has the following configuration:



## 23

where this moiety can be attached to the polymer by an ether or ester linkage.

Polymers described immediately above which are suitable for use in the compositions and methods of the present invention can be homopolymers or copolymers. One type of copolymer includes ethylene repeat units, particularly in a copolymer containing repeat units represented by Structural Formula (A) and/or Structural Formula (B).

In one embodiment of the invention, a polymer comprises repeat units represented by Structural Formula (A). In a first group of such polymers, the sum of m and p is typically two or greater. When the sum of m and p is greater than two, Z is typically a phenolic antioxidant, as described above. One preferred phenolic antioxidant is a 3,5-di-tert-butyl-4-hydroxyphenyl group, particularly when X is  $-\text{C}(\text{O})-$ . For these values of X and Z, m is preferably 2 and n and p are each 0. A second preferred antioxidant is a 3,4,5-trihydroxyphenyl group, particularly when X is  $-\text{C}(\text{O})-$ . Other preferred antioxidants are mono and di-tert-butyated-4-hydroxyphenyl groups, 4-acetoxy-3-tert-butylphenyl groups and 3-alkoxycarbonyl-2,6-dihydroxyphenyl groups (e.g., 3-propanoxycarbonyl-2,6-dihydroxyphenyl groups), particularly when X is a covalent bond.

In a second set of these polymer having repeat units represented by Structural Formula (A), m and p are each 0. When m and p are 0, n is also typically 0. For these values of m, n and p, Z is typically ascorbic acid. X is typically a covalent bond. Alternatively, Z is a 3,4,5-trihydroxyphenyl group or a 4-acetoxy-3-tert-butylphenyl group, particularly when X is  $-\text{C}(\text{O})-$ .

In another embodiment of the invention, an antioxidant polymer has repeat units represented by Structural Formula (B). For these polymers, m, n and p are each typically 0. Z is preferably a phenolic antioxidant, specifically a 3,4,5-trihydroxyphenyl, 3,5-di-tert-butyl-4-hydroxyphenyl group or a 3,5-di-tert-butyl-2-hydroxyphenyl group.

A further embodiment of the invention involves polymers that include repeat units represented by Structural Formula (C). In one group of such polymers, Y is  $-\text{O}-$  and Z is preferably ascorbic acid, particularly when k is 0. In another group, Y is  $-\text{O}-$  and Z is a phenolic antioxidant, particularly when k is 0 to 3; more preferably, k is 1. A preferred phenolic antioxidant is a 3,5-di-tert-butyl-4-hydroxyphenyl group. Other examples include of phenolic antioxidants include 4-acetoxy-3-tert-butylphenyl, 3-tert-butyl-4-hydroxyphenyl, 2,6-di-tert-butyl-4-mercaptophenyl and 2,6-di-tert-butyl-4-hydroxyphenyl groups.

In yet another embodiment of the invention, a polymer includes repeat units represented by Structural Formula (D). Typically, R' is a covalent bond or  $-\text{OH}$  in such polymers. Other typical values of R' are amide and ester linkages. Preferred Z groups can be phenolic antioxidants, as described above. For these polymers, the phenol hydroxyl group is typically para or meta to the group containing Z, more typically para.

Antioxidant polymers described immediately above which are suitable for use in the methods of the present invention have two or more repeat units, preferably greater than about five repeat units. The molecular weight of the polymers disclosed herein can be generally selected to be appropriate for the desired application. Typically, the molecular weight can be greater than about 500 atomic mass units (amu) and less than about 2,000,000 amu, greater than about 1000 amu and less than about 1,000,000 amu, greater than about 1000 amu and less than about 100,000 amu, greater than about 2,000 amu and less than about 10,000 amu, or greater than about 2,000 amu and less than about 5,000 amu.

## 24

Antioxidant polymers described immediately above which are suitable for use in the methods of the present invention can be typically insoluble in aqueous media. The solubility of the antioxidant polymers in non-aqueous media (e.g., oils) depends upon the molecular weight of the polymer, such that high molecular weight polymers can be typically sparingly soluble in non-aqueous media. When an antioxidant polymer of the invention can be insoluble in a particular medium or substrate, it can be preferably well-mixed with that medium or substrate.

In another embodiment, the first antioxidants which are suitable for use in the compositions and methods of the present invention are represented by the following structural formula:



n and m in each occurrence, independently is 0 or a positive integer. Preferably 0 to 18 inclusive.

j in each occurrence, independently is 0, 1, 2, 3 or 4.

Z' in each occurrence, independently is  $-\text{C}(\text{O})\text{O}-$ ,  $-\text{OC}(\text{O})-$ ,  $-\text{C}(\text{O})\text{NH}-$ ,  $-\text{NHC}(\text{O})-$ ,  $-\text{NH}-$ ,  $-\text{CH}=\text{N}-$ ,  $-\text{N}=\text{CH}-$ ,  $-\text{C}(\text{O})-$ ,  $-\text{O}-$ ,  $-\text{S}-$ ,  $-\text{S}-\text{S}-$ ,  $-\text{S}=\text{N}-$ ,  $-\text{N}=\text{S}-$ ,  $-\text{C}(\text{S})\text{O}-$ ,  $-\text{OC}(\text{S})-$ ,  $-\text{OP}(\text{O})$   $(\text{OR}_4)\text{O}-$ ,  $\text{OP}(\text{OR}_4)\text{O}-$ ,  $-\text{C}(\text{O})\text{OC}(\text{O})-$  or a bond. In one embodiment, Z' is  $-\text{C}(\text{O})\text{O}-$ .

R' in each occurrence, independently is C1-C6 alkyl,  $-\text{OH}$ ,  $-\text{NH}_2$ ,  $-\text{SH}$ , an optionally substituted aryl, an optionally substituted ester or



wherein at least one R' adjacent to the  $-\text{OH}$  group is an optionally substituted bulky alkyl group (e.g., butyl, sec-butyl, tert-butyl, 2-propyl, 1,1-dimethylhexyl, and the like).

R'\_1 in each occurrence, independently is C1-C6 alkyl, an optionally substituted aryl, an optionally substituted aralkyl,  $-\text{OH}$ ,  $-\text{NH}_2$ ,  $-\text{SH}$ , or C1-C6 alkyl ester wherein at least one R'\_1 adjacent to the  $-\text{OH}$  group is a bulky alkyl group (e.g., butyl, sec-butyl, tert-butyl, 2-propyl, 1,1-dimethylhexyl, and the like.).

M' is H, an optionally substituted aryl, C1-C20 linear or branched alkyl chain with or without any functional group anywhere in the chain,



25

-continued



o is 0 or a positive integer,

R'j in each occurrence, independently is —H, C1-C6 alkyl, —OH, —NH<sub>2</sub>, —SH, optionally substituted aryl, ester, or

5

In certain embodiments M' is



In certain embodiments M' is



15

wherein at least one R'j is —OH.

R'j in each occurrence, independently is —H, C1-C6 alkyl, 20 optionally substituted aryl, optionally substituted aralkyl —OH, —NH<sub>2</sub>, —SH or ester.

In another embodiment, the first antioxidants which are suitable for use in the compositions and methods of the present invention are represented by the following structural formula: 25



30

In certain embodiments, at least one R'j is



In certain embodiments n is 0.

In certain embodiments m is 1.

In certain embodiments n is 0, m is 1 and Z is —C(O)O—.

In certain embodiments n is 0, m is 1, Z is —C(O)O— and the two R'j groups adjacent to the —OH are t-butyl.

In certain embodiments n is 0, m is 1, Z is —C(O)O—, the two R'j groups adjacent to the —OH are t-butyl and M' is

X' in each occurrence, independently is —C(O)O—, —OC(O)—, —C(O)NH—, —NHC(O)—, —NH—, —CH=N—, 35 —C(O)—, —O—, —S—, —C(O)OC(O)— or a bond.

R'j is C1-C6 alkyl, —OH, —NH<sub>2</sub>, —SH, aryl, ester, or

40

wherein at least one R'j is —OH, and the values and preferred values for the remainder of the variables are as described immediately above.

In certain embodiments Z' is —C(O)O—. In certain other embodiments Z' is —OC(O)—. In certain other embodiments Z' is —C(O)NH—. In certain other embodiments Z' is —NHC(O)—. In certain other embodiments Z' is —NH—. In certain other embodiments Z' is —CH=N—. In certain other embodiments Z' is —N=CH—. In certain other embodiments Z' is —C(O)—. In certain other embodiments Z' is —O—. In certain other embodiments Z' is —S—. In certain other embodiments Z' is —S—S—. In certain other embodiments Z' is —S=N—. In certain other embodiments Z' is —N=S—. In certain other embodiments Z' is —C(S)O—. In certain other embodiments Z' is —OC(S)—. In certain other embodiments Z' is —OP(O)(OR<sub>4</sub>)O—. In certain other embodiments Z' is —OP(OR<sub>4</sub>)O—. In certain other embodiments Z' is —C(O)OC(O)—. In certain other embodiments Z' is a bond. 45

In certain embodiments both R'j groups adjacent to the —OH group is an optionally substituted bulky alkyl group. In a particular embodiment both R'j groups adjacent to the —OH group are tert-butyl. 55



In certain embodiments n is 0, m is 1, Z is —C(O)O—, the two R'j groups adjacent to the —OH are t-butyl, M' is



and the R'j in the para position is —OH.

In certain embodiments n is 0, m is 1, Z is —C(O)O—, the two R'j groups adjacent to the —OH are t-butyl, M' is



the R'j in the para position is —OH and an adjacent R'j is —OH.

27

In certain embodiments n is 0, m is 1, Z is  $-\text{C}(\text{O})\text{O}-$ , the two R' groups adjacent to the  $-\text{OH}$  are t-butyl, M' is



5

the R'2 in the para position is  $-\text{OH}$  and the two adjacent R'2 are  $-\text{OH}$ .

In certain embodiments n is 0, m is 1, Z is  $-\text{C}(\text{O})\text{O}-$ , the two R' groups adjacent to the  $-\text{OH}$  are t-butyl, M' is



10



10



10

20



20



20

25

In certain embodiments n is 0, m is 1, Z is  $-\text{C}(\text{O})\text{O}-$ , the two R' groups adjacent to the  $-\text{OH}$  are t-butyl, M' is



30



30



30

40



40



40

and R<sub>3</sub> is  $-\text{H}$ .

Specific examples of compounds and polymers which are suitable for use in the compositions and methods of the present invention are represented by one of the following structural formulas:



50



50

55



55

60



60

65

28

-continued

29  
-continued30  
-continued

In another embodiment, the first antioxidants which are suitable for use in the compositions and methods of the present invention include a macromonomer represented by Structural Formula I and I'.

I



In I, R and R<sub>1</sub>-R<sub>6</sub> are independently —H, —OH, or a C1-C10 optionally substituted linear or branched alkyl group. n is an integer from 0 to 24.

I'



## 31

In I', each of R and R<sub>1</sub>-R<sub>8</sub> are independently —H, —OH, or a C1-C10 alkyl group. n is an integer from 0 to 24. R' is —H, optionally substituted C1-C20 alkyl or optionally substituted aryl group.

In another embodiment, the first antioxidants which are suitable for use in the compositions and methods of the present invention include a macromonomer represented by Structural Formula III and an antioxidant polymer represented by Structural Formula IV. The variables are as defined above.



polymerization  
deacetylation



polymerization  
deacetylation

## 32

-continued



20 In III' and IV' each of R, and R<sub>1</sub>-R<sub>8</sub> are independently —H, —OH, or a C1-C10 alkyl group. n is an integer from 0 to 24. m is an integer equal to 2 or greater. R' is —H, optionally substituted C1-C20 alkyl or optionally substituted aryl group. In III and IV the variables are as defined above.

25 Repeat units of the antioxidant polymers as described immediately above suitable for use in the compositions and methods of the present invention include substituted benzene molecules. These benzene molecules are typically based on phenol or a phenol derivative, such that they have at least one

30 hydroxyl or ether functional group. Preferably, the benzene molecules have a hydroxyl group. The hydroxyl group can be a free hydroxyl group and can be protected or have a cleavable group attached to it (e.g., an ester group). Such cleavable groups can be released under certain conditions (e.g., changes in pH), with a desired shelf life or with a time-controlled release (e.g., measured by the half-life), which allows one to control where and/or when an antioxidant polymer can exert its antioxidant effect. The repeat units can also include analogous thiophenol and aniline derivatives, e.g., where the phenol —OH can be replaced by —SH, —NH—, and the like.

40 Substituted benzene repeat units of an antioxidant polymer as described immediately above suitable for use in the compositions and methods of the present invention are also typically substituted with a bulky alkyl group or an n-alkoxycarbonyl group. Preferably, the benzene monomers are

45 substituted with a bulky alkyl group. More preferably, the bulky alkyl group is located ortho or meta to a hydroxyl group on the benzene ring, typically ortho. A “bulky alkyl group” is defined herein as an alkyl group that is branched alpha- or beta- to the benzene ring. Preferably, the alkyl group is branched alpha to the benzene ring. More preferably, the alkyl group is branched twice alpha to the benzene ring, such as in

50 a tert-butyl group. Other examples of bulky alkyl groups include isopropyl, 2-butyl, 3-pentyl, 1,1-dimethylpropyl, 1-ethyl-1-methylpropyl and 1,1-diethylpropyl. The bulky alkyl groups are preferably unsubstituted, but they can be substituted with a functional group that does not interfere with the antioxidant activity of the molecule or the polymer. Straight chained alkoxy carbonyl groups include methoxy carbonyl, ethoxycarbonyl, n-propoxycarbonyl, n-butoxycarbonyl and n-pentoxy carbonyl. n-propoxycarbonyl is a preferred group. Similar to the bulky alkyl groups, n-alkoxycarbonyl groups are optionally substituted with a functional group that does not interfere with the antioxidant activity of the molecule or the polymer.

60 Antioxidant polymers as described immediately above 65 suitable for use in the compositions and methods of the present invention have two or more repeat units, preferably greater than about five repeat units. The molecular weight of

the polymers disclosed herein can be generally selected to be appropriate for the desired application. Typically, the molecular weight can be greater than about 500 atomic mass units (amu) and less than about 2,000,000 amu, greater than about 1000 amu and less than about 100,000, greater than about 2,000 amu and less than about 10,000, or greater than about 2,000 amu and less than about 5,000 amu.

Antioxidant polymers as described immediately above suitable for use in the compositions and methods of the present invention can be either homopolymers or copolymers. A copolymer preferably contains two or more or three or more different repeating monomer units, each of which has varying or identical antioxidant properties. The identity of the repeat units in a copolymer can be chosen to modify the antioxidant properties of the polymer as a whole, thereby giving a polymer with tunable properties. The second, third and/or further repeat units in a copolymer can be either a synthetic or natural antioxidant.

Antioxidant polymers as described immediately above suitable for use in the compositions and methods of the present invention are typically insoluble in aqueous media. The solubility of the antioxidant polymers in non-aqueous media (e.g., oils) depends upon the molecular weight of the polymer, such that high molecular weight polymers are typically sparingly soluble in non-aqueous media. When an antioxidant polymer of the invention can be insoluble in a particular medium or substrate, it can be preferably well-mixed with that medium or substrate.

Antioxidant polymers as described immediately above suitable for use in the compositions and methods of the present invention can be branched or linear, but are preferably linear. Branched antioxidant polymers can only be formed from benzene molecules having three or fewer substituents (e.g., three or more hydrogen atoms).

In another embodiment, the antioxidants which are suitable for use in the compositions and methods of the present invention include macromolecule antioxidants represented by Structural Formula J or J':



In J, R and R<sub>1</sub>-R<sub>6</sub> are independently —H, —OH, or a C1-C10 optionally substituted linear or branched alkyl group. n is an integer from 0 to 24.



In J' Each R<sub>a</sub> is independently an optionally substituted alkyl. Each R<sub>b</sub> is independently an optionally substituted alkyl. Each R<sub>c</sub> is independently an optionally substituted alkyl or an optionally substituted alkoxycarbonyl. R<sub>x</sub> is —H or an optionally substituted alkyl. R<sub>y</sub> is —H or an optionally

substituted alkyl. Each R' is independently —H or an optionally substituted alkyl. R" is —H, an optionally substituted alkyl, an optionally substituted aryl or an optionally substituted aralkyl. n is an integer from 1 to 10. m is an integer from 1 to 10. s is an integer from 0 to 5. t is an integer from 0 to 4. u is an integer from 1 to 4. With the proviso that when n is 1, then either ring C is not:



s is not 0, or R" is not —H.

Specific examples of macromolecule antioxidants represented by Structural Formula J which are suitable for use in the compositions and methods of the present invention are represented by one of the following structural formulas:



35

-continued



36

In one embodiment the variables in  $J^1$  are as described as follows:

Each  $R_a$  is independently an optionally substituted alkyl. In one embodiment, each  $R_a$  is independently a C1-C20 alkyl. In another embodiment, each  $R_a$  is independently a C1-C10 alkyl. In another embodiment, each  $R_a$  is independently selected from the group consisting of:



In another embodiment, the antioxidants which are suitable for use in the compositions and methods of the present invention include macromolecular antioxidants represented by structural formula  $J^1$ :



Each  $R_a$  is independently an optionally substituted alkyl. Each  $R_b$  is independently an optionally substituted alkyl. Each  $R_c$  is independently an optionally substituted alkyl or an optionally substituted alkoxy carbonyl.  $R_x$  is  $-H$  or an optionally substituted alkyl.  $R_y$  is  $-H$  or an optionally substituted alkyl. Each  $R'$  is independently  $-H$  or an optionally substituted alkyl.  $R''$  is  $-H$ , an optionally substituted alkyl, an optionally substituted aryl or an optionally substituted aralkyl.  $n$  is an integer from 1 to 10.  $m$  is an integer from 1 to 10.  $s$  is an integer from 0 to 5.  $t$  is an integer from 0 to 4.  $u$  is an integer from 1 to 4. With the proviso that when  $n$  is 1, then either ring C is not:



is not 0, or  $R''$  is not  $-H$ .

37

In another embodiment  $R_a$  is:Each  $R_b$  is independently an optionally substituted alkyl.Each  $R_c$  is independently an optionally substituted alkyl or an optionally substituted alkoxy carbonyl. In one embodiment, each  $R_c$  is independently a C1-C10 alkyl.Each  $R_x$  is —H or an optionally substituted alkyl.  $R_y$  is —H or an optionally substituted alkyl. In one embodiment,  $R_x$  and  $R_y$  are —H.Each  $R'$  is independently —H or an optionally substituted alkyl. In one embodiment, one  $R'$  is —H. In another embodiment, both  $R'$  are —H.Each  $R''$  is —H, an optionally substituted alkyl, an optionally substituted aryl or an optionally substituted aralkyl. In one embodiment,  $R''$  is —H, a C1-C20 alkyl or an optionally substituted aralkyl. In another embodiment,  $R''$  is —H, a C1-C10 alkyl or a substituted benzyl group. In yet another embodiment,  $R''$  is —H. In yet another embodiment,  $R''$  is:In yet another embodiment  $R''$  is selected from the group consisting of:

38

-continued

In yet another embodiment  $R''$  is:

35 n is an integer from 1 to 10. In one embodiment, n is an integer from 1 to 6. In another embodiment, n is 1. In yet another embodiment, n is 2. In yet another embodiment, n is 3. In yet another embodiment, n is 4.

m is an integer from 1 to 10. In one embodiment, m is 1 or 40 2. In another embodiment, m is 1.

s is an integer from 0 to 5. In one embodiment, s is 0 or 1. In another embodiment, s is 0.

t is an integer from 0 to 4. In one embodiment, t is 0.

u is an integer from 1 to 4. In one embodiment, u is 1 or 2.

45 In certain embodiments for antioxidants represented by  $J^1$ , when n is 1, the either ring C is not:50 s is not 0, or  $R''$  is not —H.60 In one embodiment in  $J^1$ :Each  $R_a$  is independently a C1-C20 alkyl. Each  $R_c$  is independently a C1-C10 alkyl.  $R''$  is —H, a C1-C20 alkyl or an optionally substituted aralkyl, and the remainder of the variables are as described above for structural formula (I).65 In another embodiment in  $J^1$ : one  $R'$  is —H, t is 0,  $R_x$  and  $R_y$  are —H and the compounds are represented by structural formula  $J^2$ :

39



and the remainder of the variables are as described in the immediately preceding paragraph or for structural formula J<sup>1</sup>

In another embodiment in  $J^2$ :

$m$  is 1 or 2.

$s$  is 0 or 1.

$u$  is 1 or 2, and the remainder of the variables are as described in the immediately preceding paragraph or for  $J^1$ .

In another embodiment in  $J^2$ : both  $R'$  are  $-\bar{H}$  and  $m$  is 1 and the compounds are represented by structural formula  $J^3$ :



and the remainder of the variables are as described in the immediately preceding paragraph or for structural formula  $J^1$  35 or  $J^2$ .

In another embodiment in  $J^3$ :

Each  $R_a$  is independently a C1-C10 alkyl.

R" is —H, a C1-C10 alkyl or a substituted benzyl group.

*n* is an integer from 1 to 6, and the remainder of the variables are as described in the immediately preceding paragraph or for structural formula  $J^1$  or  $J^2$ .

In another embodiment in  $J^3$ : n is 1, s is 0 and  $R''$  is —H and the compounds are represented by structural formula  $J^4$ :



with the proviso that ring C is not:



and the remainder of the variables are as described above for structural formula  $J^1$ ,  $J^2$ , or  $J^3$ .

40

In certain embodiments of the present invention the anti-oxidants which are suitable for use in the compositions and methods of the present invention include structural formula J<sup>3</sup> or J<sup>4</sup> represented by the following structural formulas:



55 In another embodiment in J<sup>3</sup>: n is 1 and the compounds are represented by structural formula J<sup>5</sup>:



and the remainder of the variables are as described above for structural formula  $J^1$ ,  $J^2$ , or  $J^3$ .

**41**

In another embodiment of the present invention for compounds represented by structural formula J<sup>3</sup>: s is 0 and the compounds are represented by structural formula J<sup>6</sup>.



and the remainder of the variables are as described above for structural formula J<sup>1</sup>, J<sup>2</sup>, or J<sup>3</sup>.

In another embodiment of the present invention for compounds represented by structural formula J<sup>3</sup>: R" is —H and the compounds are represented by structural formula J<sup>7</sup>:

**42**

and the remainder of the variables are as described above for structural formula J<sup>1</sup>, J<sup>2</sup> or J<sup>3</sup>.

In certain embodiments of the present invention the compounds represented by structural formula J<sup>3</sup>, J<sup>5</sup>, J<sup>6</sup> or J<sup>7</sup> are represented by the following structural formulas:



-continued



**45****46**

-continued



-continued



-continued



In another embodiment of the present invention for compounds represented by structural formula  $J^3$ :  $R''$  is  $-H$  and  $n$  is 1 and the compounds are represented by structural formula  $J^8$ :

and the remainder of the variables are as described above for structural formula  $J^1$ ,  $J^2$  or  $J^3$ .

60

 $J^8$ 

In certain embodiments of the present invention the compounds represented by structural formula  $J^3$  or  $J^8$  are represented by the following structural formulas:

65

51



52

53

In another embodiment of the present invention for compounds represented by structural formula  $J^3$ :  $s$  is 0 and  $R''$  is  $-\text{H}$  and the compounds are represented by structural formula  $J^9$ :

54

and the remainder of the variables are as described above for structural formula  $J^1$ ,  $J^2$  or  $J^3$ .

5



In certain embodiments of the present invention the compounds represented by structural formula  $J^3$  or  $J^9$  are represented by the following structural formulas:



**55**

In another embodiment of the present invention for compounds represented by structural formula J<sup>3</sup>: s is 0 and n is 0 and the compounds are represented by structural formula J<sup>10</sup>:



and the remainder of the variables are as described above for structural formula J<sup>1</sup>, J<sup>2</sup> or J<sup>3</sup>.

In certain embodiments of the present invention the compounds represented by structural formula J<sup>3</sup> or J<sup>10</sup> are represented by the following structural formulas:

**56**

-continued



In another embodiment of the present invention the antioxidants which are suitable for use in the compositions and methods of the present invention include compounds represented by the following structural formulas:



-continued



59

60

-continued



**61****62**

-continued



63



-continued

64



In another embodiment, the first antioxidants which are suitable for use in the compositions and methods of the present invention include alkylated antioxidant macromolecules having formula K:



—OH group is a bulky alkyl group (e.g., butyl, sec-butyl, tert-butyl, 2-propyl, 1,1-dimethylhexyl, and the like); and  
 R<sub>2</sub> is H, C<sub>1-6</sub> alkyl, aryl, aralkyl, —OH, —NH<sub>2</sub>, or —SH  
 35 wherein at least one R<sub>1</sub> adjacent to the —OH group is a bulky alkyl group (e.g., butyl, sec-butyl, tert-butyl, 2-propyl, 1,1-dimethylhexyl, and the like);

X is —C(O)O—, —OC(O)—, —C(O)NH—, —NHC(O)—, —NH—, —CH=N—, —C(O)—, —O—, —S—, —C(O)OC(O)—, or a bond;

40 M is H, aryl, C-1 to C-20 linear or branched alkyl chain with or without any functional group anywhere in the chain, or



wherein, independently for each occurrence, n and m are integers from 0 to 6, inclusive;  
 Z is —C(O)O—, —OC(O)—, —C(O)NH—, —NHC(O)—, —NH—, —CH=N—, —C(O)—, —O—, —S—, —C(O)OC(O)—, or a bond;

50 R is H, C<sub>1-6</sub> alkyl, —OH, —NH<sub>2</sub>, —SH, aryl, aralkyl, or



wherein at least one R adjacent to the —OH group is a bulky alkyl group (e.g., butyl, sec-butyl, tert-butyl, 2-propyl, 1,1-dimethylhexyl, and the like);

R<sub>1</sub> is H, C<sub>1-6</sub> alkyl, aryl, alkylaryl, —OH, —NH<sub>2</sub>, —SH, or C1-C6 alkyl ester wherein at least one R<sub>1</sub> adjacent to the

55 wherein m and each R is independently as described above; wherein

R<sub>2</sub> is H, C<sub>1-6</sub> alkyl, —OH, —NH<sub>2</sub>, —SH, aryl, ester, or



60 In certain embodiment, at least one R<sub>2</sub> is —OH and n, Z, and each R<sub>1</sub> are independently as described above.

65

In various embodiments, for compounds of formula K, Z is  $-\text{OC(O)}-$ . In another embodiment, Z is  $-\text{C(O)O}-$ . In another embodiment, Z is  $-\text{C(O)NH}-$ . In another embodiment, Z is  $-\text{NHC(O)}-$ . In another embodiment, Z is  $-\text{NH}-$ . In another embodiment, Z is  $-\text{CH=N}-$ . In another embodiment, Z is  $-\text{C(O)}-$ . In another embodiment, Z is  $-\text{C(O)OC(O)}-$ . In another embodiment, Z is a bond.

In another embodiment, for compounds of formula K, both R groups adjacent to  $-\text{OH}$  are bulky alkyl groups (e.g., butyl, sec-butyl, tert-butyl, 2-propyl, 1,1-dimethylhexyl, and the like). In another embodiment, both R groups are tert-butyl.

In another embodiment, for compounds of formula K, M is



In another embodiment, for compounds of formula K, at least one R is



In another embodiment for compounds of formula K, n is 0.

In another embodiment, for compounds of formula K, m is 0.

1. In another embodiment, for compounds of formula K, n is 0 and m is 1.

In another embodiment, for compounds of formula K, n is 0, m is 1, and Z is  $-\text{C(O)O}-$ .

In another embodiment, for compounds of formula K, n is 0, m is 1, Z is  $-\text{C(O)O}-$ , and the two R groups adjacent to the OH are tert-butyl.

In another embodiment, for compounds of formula K, n is 0, m is 1, Z is  $-\text{C(O)O}-$ , the two R groups adjacent to the OH are t-butyl, and M is



In another embodiment, for compounds of formula K, n is 0, m is 1, Z is  $-\text{C(O)O}-$ , the two R groups adjacent to the OH are t-butyl, M is



and the R2 in the para position is OH.

66

In another embodiment, for compounds of formula K, n is 0, m is 1, Z is  $-\text{C(O)O}-$ , the two R groups adjacent to the OH are t-butyl, M is



the R2 in the para position is OH, and an adjacent R2 is OH.

15 In another embodiment, for compounds of formula K, n is 0, m is 1, Z is  $-\text{C(O)O}-$ , the two R groups adjacent to the OH are t-butyl, M is



the R2 in the para position is OH, and the two adjacent R2 groups are OH.

30 In one embodiment the antioxidant suitable for use in the compounds and methods of the present invention are compounds represented Structural Formula K<sup>1</sup>:



40 35 45 50 55 60 65 70 75 80 85 90 95 100

Z is  $-\text{C(O)NR}'$ ,  $-\text{NR'C(O)}$ ,  $-\text{NR}'$ ,  $-\text{CR}'=\text{N}$ ,  $-\text{C(O)}$ ,  $-\text{C(O)O}$ ,  $-\text{OC(O)}$ ,  $-\text{O}$ ,  $-\text{S}$ ,  $-\text{C(O)OC(O)}$  or a bond. Each R' is independently  $-\text{H}$  or optionally substituted alkyl. Each R is independently an optionally substituted alkyl, optionally substituted aryl, optionally substituted alkoxy carbonyl, optionally substituted ester,  $-\text{OH}$ ,  $-\text{NH}_2$ ,  $-\text{SH}$ , or  $\text{OR}'$ .



Each R1 is independently an optionally substituted alkyl, optionally substituted aryl, optionally substituted alkoxy carbonyl, optionally substituted ester,  $-\text{OH}$ ,  $-\text{NH}_2$  or  $-\text{SH}$ . Each R2 is independently an optionally substituted alkyl, optionally substituted aryl, optionally substituted alkoxy carbonyl, optionally substituted ester,  $-\text{OH}$ ,  $-\text{NH}_2$  or  $-\text{SH}$ . X is  $-\text{C(O)O}$ ,  $-\text{OC(O)}$ ,  $-\text{C(O)NR}'$ ,  $-\text{NR'C(O)}$ ,  $-\text{NR}'$ ,  $-\text{CH=N}$ ,  $-\text{C(O)}$ ,  $-\text{O}$ ,  $-\text{S}$ ,  $-\text{NR}'$  or  $-\text{C(O)OC(O)}$ . M is an alkyl or



Each n and m are independently integers from 0 to 6. Each s, q and u are independently integers from 0 to 4. In certain embodiments M is not



when X is  $-\text{C}(\text{O})\text{O}-$  or  $-\text{OC}(\text{O})-$ .

In certain embodiments for compounds represented by Structural Formula K<sup>1</sup>:

Z is  $-\text{C}(\text{O})\text{NR}'-$ ,  $-\text{NR}'\text{C}(\text{O})-$ ,  $-\text{NR}'-$ ,  $-\text{CR}'=\text{N}-$ ,  $-\text{C}(\text{O})-$ ,  $-\text{C}(\text{O})\text{O}-$ ,  $-\text{OC}(\text{O})-$ ,  $-\text{O}-$ ,  $-\text{S}-$ ,  $-\text{C}(\text{O})\text{OC}(\text{O})-$  or a bond. In certain other embodiments Z is  $-\text{C}(\text{O})\text{O}-$ ,  $-\text{OC}(\text{O})-$ ,  $-\text{C}(\text{O})\text{NH}-$ ,  $-\text{NHC}(\text{O})-$ ,  $-\text{NH}-$ ,  $-\text{O}-$  or  $-\text{C}(\text{O})-$ . In certain other embodiments, Z is  $-\text{C}(\text{O})\text{NH}-$  or  $-\text{NHC}(\text{O})-$ . Optionally, Z is not  $-\text{C}(\text{O})\text{O}-$ ,  $-\text{OC}(\text{O})-$ ,  $-\text{O}-$  or  $-\text{NH}-$ . In various embodiments, the present invention relates to a compound of Structural Formula 1 and the attendant definitions, wherein Z is  $-\text{OC}(\text{O})-$ . In another embodiment, Z is  $-\text{C}(\text{O})\text{O}-$ . In another embodiment, Z is  $-\text{C}(\text{O})\text{NH}-$ . In another embodiment, Z is  $-\text{NHC}(\text{O})-$ . In another embodiment, Z is  $-\text{NH}-$ . In another embodiment, Z is  $-\text{CH}=\text{N}-$ . In another embodiment, Z is  $-\text{C}(\text{O})-$ . In another embodiment, Z is  $-\text{O}-$ . In another embodiment, Z is  $-\text{C}(\text{O})\text{OC}(\text{O})-$ . In another embodiment, Z is a bond.

Each R' is independently  $-\text{H}$  or optionally substituted alkyl. In certain other embodiments R' is  $-\text{H}$  or an alkyl group. In certain other embodiments R' is  $-\text{H}$  or a C1-C10 alkyl group. In certain other embodiments R' is  $-\text{H}$ .

Each R is independently an optionally substituted alkyl, optionally substituted aryl, optionally substituted alkoxy carbonyl, optionally substituted ester,  $-\text{OH}$ ,  $-\text{NH}_2$ ,  $-\text{SH}$ , or



In certain other embodiments, each R is independently an optionally substituted alkyl or optionally substituted alkoxy carbonyl. In certain other embodiment each R is independently an alkyl or alkoxy carbonyl. In certain other embodiments each R is independently a C1-C6 alkyl or a C1-C6 alkoxy carbonyl. In certain other embodiments each R is independently tert-butyl or propoxycarbonyl. In certain other embodiments each R is independently an alkyl group. In certain embodiments each R is independently a bulky alkyl group. Suitable examples of bulky alkyl groups include butyl, sec-butyl, tert-butyl, 2-propyl, 1,1-dimethylhexyl, and the

like. In certain embodiments each R is tert-butyl. In certain embodiments at least one R adjacent to the  $-\text{OH}$  group is a bulky alkyl group (e.g., butyl, sec-butyl, tert-butyl, 2-propyl, 1,1-dimethylhexyl, and the like). In certain other embodiments both R groups adjacent to  $-\text{OH}$  are bulky alkyl groups (e.g., butyl, sec-butyl, tert-butyl, 2-propyl, 1,1-dimethylhexyl, and the like). In another embodiment, both R groups are tert-butyl. In another embodiment, both R groups are tert-butyl adjacent to the OH group.

10 Each R<sub>1</sub> is independently an optionally substituted alkyl, optionally substituted aryl, optionally substituted alkoxy carbonyl, optionally substituted ester,  $-\text{OH}$ ,  $-\text{NH}_2$  or  $-\text{SH}$ . In certain other embodiments, each R<sub>1</sub> is independently an optionally substituted alkyl or optionally substituted alkoxy carbonyl. In certain other embodiment each R<sub>1</sub> is independently an alkyl or alkoxy carbonyl. In certain other embodiments each R<sub>1</sub> is independently a C1-C6 alkyl or a C1-C6 alkoxy carbonyl. In certain other embodiments each R<sub>1</sub> is independently tert-butyl or propoxycarbonyl. In certain other 15 embodiments each R<sub>1</sub> is independently an alkyl group. In certain embodiments each R<sub>1</sub> is independently a bulky alkyl group. Suitable examples of bulky alkyl groups include butyl, sec-butyl, tert-butyl, 2-propyl, 1,1-dimethylhexyl, and the like. In certain embodiments each R<sub>1</sub> is tert-butyl. In certain 20 embodiments at least one R<sub>1</sub> adjacent to the  $-\text{OH}$  group is a bulky alkyl group (e.g., butyl, sec-butyl, tert-butyl, 2-propyl, 1,1-dimethylhexyl, and the like). In certain other embodiments both R<sub>1</sub> groups adjacent to  $-\text{OH}$  are bulky alkyl groups (e.g., butyl, sec-butyl, tert-butyl, 2-propyl, 1,1-dimethylhexyl, and the like). In another embodiment, both R<sub>1</sub> groups are tert-butyl. In another embodiment, both R<sub>1</sub> groups are tert-butyl adjacent to the OH group.

Each R<sub>2</sub> is independently an optionally substituted alkyl, optionally substituted aryl, optionally substituted alkoxy carbonyl, optionally substituted ester,  $-\text{OH}$ ,  $-\text{NH}_2$  or  $-\text{SH}$ . In certain other embodiments, each R<sub>2</sub> is independently an optionally substituted alkyl or optionally substituted alkoxy carbonyl. In certain other embodiment each R<sub>2</sub> is independently an alkyl or alkoxy carbonyl. In certain other embodiments each R<sub>2</sub> is independently an optionally substituted alkyl. In certain other embodiment each R<sub>2</sub> is independently an alkyl. In certain other embodiments each R<sub>2</sub> is independently a C1-C10 alkyl. In certain other embodiments each R<sub>2</sub> is independently a C1-C6 alkyl. In certain other embodiments each R<sub>2</sub> is independently a bulky alkyl group or a straight 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025

69

Each n and m are independently integers from 0 to 6. In certain embodiments each n and m are independently integers from 0 to 2.

In another embodiment, the antioxidant suitable for use in the compositions and methods of the present invention is represented by a compound of Structural Formula K<sup>1</sup> wherein n is 0.

In another embodiment, the antioxidant suitable for use in the compositions and methods of the present invention is represented by a compound of Structural Formula K<sup>1</sup> wherein m is 1.

In another embodiment, the antioxidant suitable for use in the compositions and methods of the present invention is represented by a compound of Structural Formula K<sup>1</sup> and the attendant definitions, wherein n is 0 and m is 1.

In another embodiment, the antioxidant suitable for use in the compositions and methods of the present invention is represented by a compound of Structural Formula K<sup>1</sup> wherein n is 0, m is 1, and Z is —C(O)O—.

In another embodiment, the antioxidant suitable for use in the compositions and methods of the present invention is represented by a compound of Structural Formula K<sup>1</sup> wherein n is 0, m is 1, Z is —C(O)O—, and the two R groups adjacent to the OH are tert-butyl.

10

70

Each s, q and u are independently integers from 0 to 4. In certain embodiments, each s and q are independently integers from 0 to 2. In certain embodiments, s is 2.

In certain embodiments for compounds represented by Structural Formula K<sup>1</sup> M is not



20 when X is —C(O)O— or —OC(O)—.

In a sixth embodiment of the present invention directed to a compound represented by Structural Formula K<sup>1</sup>, the compound is represented by a Structural Formula selected from:



-continued



-continued



In another embodiment, the antioxidants which are suitable for use in the compositions and methods of the present invention include alkylated antioxidant macromolecules having formula L.



where M is C1 to C20-linear or branched alkyl chains.

In another embodiment the antioxidants which are suitable for use in the compositions and methods of the present invention are alkylated antioxidant macromolecules having formula A:



wherein, independently for each occurrence:

n and m are integers from 0 to 6, inclusive;

Z is  $-\text{C}(\text{O})\text{O}-$ ,  $-\text{OC}(\text{O})-$ ,  $-\text{C}(\text{O})\text{NH}-$ ,  $-\text{NHC}(\text{O})-$ ,  $-\text{NH}-$ ,  $-\text{CH}=\text{N}-$ ,  $-\text{C}(\text{O})-$ ,  $-\text{O}-$ ,  $-\text{S}-$ ,  $-\text{C}(\text{O})\text{OC}(\text{O})-$ , or a bond;

R is H, C<sub>1-6</sub> alkyl,  $-\text{OH}$ ,  $-\text{NH}_2$ ,  $-\text{SH}$ , aryl, ester, or



wherein at least one R adjacent to the  $-\text{OH}$  group is a bulky alkyl group (e.g., butyl, sec-butyl, tert-butyl, 2-propyl, 1,1-dimethylhexyl, and the like);

R<sub>1</sub> is H, C<sub>1-6</sub> alkyl, aryl, aralkyl,  $-\text{OH}$ ,  $-\text{NH}_2$ ,  $-\text{SH}$ , or C<sub>1-C<sub>6</sub></sub> alkyl ester wherein at least one R<sub>1</sub> adjacent to the  $-\text{OH}$  group is a bulky alkyl group (e.g., butyl, sec-butyl, tert-butyl, 2-propyl, 1,1-dimethylhexyl, and the like); and

20 R<sub>2</sub> is H, C<sub>1-6</sub> alkyl, aryl, aralkyl,  $-\text{OH}$ ,  $-\text{NH}_2$ ,  $-\text{SH}$ , or ester, wherein at least one R<sub>1</sub> adjacent to the  $-\text{OH}$  group is a bulky alkyl group (e.g., butyl, sec-butyl, tert-butyl, 2-propyl, 1,1-dimethylhexyl, and the like);

25 X is  $-\text{C}(\text{O})\text{O}-$ ,  $-\text{OC}(\text{O})-$ ,  $-\text{C}(\text{O})\text{NH}-$ ,  $-\text{NHC}(\text{O})-$ ,  $-\text{O}-$ ,  $-\text{S}-$ ,  $-\text{C}(\text{O})\text{OC}(\text{O})-$ , or a bond;

30 M is H, aryl, C<sub>1</sub> to C-20 linear or branched alkyl chain with or without any functional group anywhere in the chain, or



35 In one embodiment, the first antioxidants which are suitable for use in the compositions and methods of the present invention are sterically hindered phenol and phosphite based compounds, represented by a formula selected from I-III:

40 Specific examples of compounds which are suitable for use in the compositions and methods of the present invention are represented by one of the following structural formulas:



75



In one embodiment, the first antioxidants which are suitable for use in the compositions and methods of the present invention are sterically hindered phenol and phosphate based compounds, represented by a formula selected from O, P and Q.



R is:



independently an optionally substituted alkyl. In another embodiment, each R<sub>1</sub> and R<sub>2</sub> are independently a linear or branched C<sub>1</sub>-C<sub>6</sub> alkyl.

In one embodiment R is:



In another embodiment R is:



In yet another embodiment R is:



R<sub>1</sub> and R<sub>2</sub> in each occurrence, independently is an optionally substituted alkyl, optionally substituted aryl or optionally substituted aralkyl. In one embodiment, each R<sub>1</sub> and R<sub>2</sub> are

X and Y in each occurrence independently is a bond, —O—, —NH—, —C(O)NH—, —NHC(O)—, —C(O)O—,

—OC(O)— or —CH<sub>2</sub>—. In one embodiment, X and Y in each occurrence independently is a bond or —CH<sub>2</sub>—. In another embodiment, X and Y in each occurrence independently is a bond, —O— or —CH<sub>2</sub>—. In yet another embodiment, X and Y in each occurrence independently is a bond, —NH— or —CH<sub>2</sub>—. In yet another embodiment, X and Y in each occurrence independently is a bond, —C(O)NH— or —CH<sub>2</sub>—. In yet another embodiment, X and Y in each occurrence independently is a bond, —NHC(O)—, or —CH<sub>2</sub>—. In yet another embodiment, X and Y in each occurrence independently is a bond, —C(O)O— or —CH<sub>2</sub>—. In yet another embodiment, X and Y in each occurrence independently is a bond, —OC(O)— or —CH<sub>2</sub>—.

n and m in each occurrence independently is 0 or a positive integer. In one embodiment, n and m in each occurrence independently is 0 to 18. In another embodiment, n and m in each occurrence independently is 0 to 12. In yet another embodiment, n and m are in each occurrence independently is 0 to 6.

i and j in each occurrence independently is 0, 1, 2, 3 or 4. In one embodiment i and j in each occurrence independently is 0, 1 or 2. In a particular embodiment, i is 0. In another particular embodiment j is 2.

R" is an optionally substituted alkyl. In one embodiment R" is C1-C6 alkyl.

In a particular embodiment, for compounds represented by structural formulas O, P and Q, R is:



and n and m in each occurrence independently is 0 to 12, and the remainder of the variables are as described above for structural formulas O, P and Q.

In another particular embodiment, for compounds represented by structural formulas O, P and Q, R, n and m are as described immediately above, and R<sub>1</sub> and R<sub>2</sub> in each occurrence, independently is an optionally substituted alkyl; i and j in each occurrence independently is 0, 1 or 2; and the remainder of the variables are as described above for structural formulas O, P and Q.

In yet another particular embodiment, for compounds represented by structural formulas O, P and Q, R<sub>1</sub>, R<sub>2</sub>, i and j are as described immediately above, and R is:



n and m in each occurrence, independently is 0 to 6; and the remainder of the variables are as described above for structural formulas O, P and Q.

In another particular embodiment, for compounds represented by structural formulas O, P and Q, R<sub>1</sub>, R<sub>2</sub>, i, j, R, n and m are as described immediately above, and

X and Y in each occurrence, independently is a bond or —CH<sub>2</sub>—; and the remainder of the variables are as described above for structural formulas O, P and Q.

In another particular embodiment, for compounds represented by structural formulas O, P and Q, R<sub>1</sub>, R<sub>2</sub>, i, j, R, n and m are as described immediately above, and X and Y in each occurrence, independently is a bond, —O— or —CH<sub>2</sub>—; and the remainder of the variables are as described above for structural formulas O, P and Q.

In another particular embodiment, for compounds represented by structural formulas O, P and Q, R<sub>1</sub>, R<sub>2</sub>, i, j, R, n and m are as described immediately above, and X and Y in each occurrence, independently is a bond, —NH— or —CH<sub>2</sub>—; and the remainder of the variables are as described above for structural formulas O, P and Q.

In another particular embodiment, for compounds represented by structural formulas O, P and Q, R<sub>1</sub>, R<sub>2</sub>, i, j, R, n and m are as described immediately above, and X and Y in each occurrence, independently is a bond, —C(O)NH— or —CH<sub>2</sub>—; and the remainder of the variables are as described above for structural formulas O, P and Q.

In another particular embodiment, for compounds represented by structural formulas O, P and Q, R<sub>1</sub>, R<sub>2</sub>, i, j, R, n and m are as described immediately above, and X and Y in each occurrence, independently is a bond, —NHC(O)—, or —CH<sub>2</sub>—; and the remainder of the variables are as described above for structural formulas O, P and Q.

In another particular embodiment, for compounds of the present invention represented by structural formulas O, P and Q, R<sub>1</sub>, R<sub>2</sub>, i, j, R, n and m are as described immediately above, and X and Y in each occurrence, independently is a bond, —C(O)O— or —CH<sub>2</sub>—; and the remainder of the variables are as described above for structural formulas O, P and Q.

In another particular embodiment, for compounds of the present invention represented by structural formulas O, P and Q, R<sub>1</sub>, R<sub>2</sub>, i, j, R, n and m are as described immediately above,

79

and X and Y in each occurrence, independently is a bond, —OC(O)— or —CH<sub>2</sub>—; and the remainder of the variables are as described above for structural formulas O, P and Q.

In an additional embodiment, for formulas O, P and Q R is:



n and m in each occurrence, independently is 0 or a positive integer. In one embodiment, n and m in each occurrence, independently is 0 to 18. In another embodiment, n and m in each occurrence, independently is 0 to 12. In yet another embodiment, n and m in each occurrence, independently is 0 to 6.

i and j in each occurrence, independently is 0, 1, 2, 3 or 4. In one embodiment, i and j in each occurrence, independently is 0, 1 or 2. In a particular embodiment, i is 0. In another particular embodiment, j is 2.

Z' is —C(O)O—, —OC(O)—, —C(O)NH—, —NHC(O)—, —NH—, —CH=N—, —C(O)—, —O—, —S—, —C(O)OC(O)— or a bond. In one embodiment, Z' is —C(O)O—. In another embodiment, Z' is —OC(O)—. In yet another embodiment, Z' is —C(O)NH—. In yet another embodiment, Z' is —NHC(O)—. In yet another embodiment, Z' is —NH—. In yet another embodiment, Z' is —CH=N—. In yet another embodiment, Z' is —C(O)—. In yet another embodiment, Z' is —O—. In yet another embodiment, Z' is —S—. In yet another embodiment, Z' is —C(O)OC(O)—. In yet another embodiment, Z' is a bond.

R' is an optionally substituted C1-C6 alkyl, —OH, —NH<sub>2</sub>, —SH, an optionally substituted aryl, an ester or



wherein at least one R' adjacent to the —OH group is an optionally substituted bulky alkyl group (e.g., butyl, sec-butyl, tert-butyl, 2-propyl, 1,1-dimethylhexyl, and the like).

R'1 is an optionally substituted C1-C6 alkyl, an optionally substituted aryl, an optionally substituted aralkyl, —OH, —NH<sub>2</sub>, —SH, or C1-C6 alkyl ester wherein at least one R<sub>1</sub> adjacent to the —OH group is a bulky alkyl group (e.g., butyl, sec-butyl, tert-butyl, 2-propyl, 1,1-dimethylhexyl, and the like.).

R'2 is an optionally substituted C1-C6 alkyl, an optionally substituted aryl, an optionally substituted aralkyl, —OH, —NH<sub>2</sub>, —SH, or ester.

X' is —C(O)O—, —OC(O)—, —C(O)NH—, —NHC(O)—, —NH—, —CH=N—, —C(O)—, —O—, —S—, —C(O)OC(O)— or a bond. In one embodiment X' is —C(O)O—. In another embodiment X' is —OC(O)—. In yet another embodiment X' is —C(O)NH—. In yet another embodiment

80

X' is —NHC(O)—. In yet another embodiment X' is —NH—. In yet another embodiment X' is —CH=N—. In yet another embodiment X' is —C(O)—. In yet another embodiment X' is —O—. In yet another embodiment X' is —S—. In yet another embodiment X' is —C(O)OC(O)—. In yet another embodiment X' is a bond.

M' is H, an optionally substituted aryl, an optionally substituted C1-C20 linear or branched alkyl chain with or without any functional group anywhere in the chain, or



o is 0 or a positive integer. Preferably o is 0 to 18. More preferably o is 0 to 12. Even more preferably o is 0 to 6.

In yet another embodiment, for formulas O, P and Q R is:



R'2 is C1-C6 alkyl, —OH, —NH<sub>2</sub>, —SH, aryl, ester, aralkyl or



wherein at least one R'2 is —OH, and the values and preferred values for the remainder of the variables for R are as described immediately above.

In yet another embodiment, the present invention relates to a compound of formula O, P and Q, wherein M is



Wherein p is 0, 1, 2, 3 or 4; and the values and preferred values for the remainder of the variables are as described above for formulas O, P and Q.

Specific examples of compounds which are suitable for use in the compositions and methods of the present invention are represented by one of the following structural formulas:

**81****82**

and



83

In another embodiment, the first antioxidants which are suitable for use in the compositions and methods of the present invention are represented by a structural formula selected from 1-6:



85

In yet another particular embodiment R is:



R<sub>1</sub> and R<sub>2</sub> in each occurrence, independently is an optionally substituted alkyl, optionally substituted aryl or optionally substituted aralkyl. In one embodiment, each R<sub>1</sub> and R<sub>2</sub> in each occurrence, independently is an optionally substituted alkyl. In another embodiment, each R<sub>1</sub> and R<sub>2</sub> in each occurrence, independently is a C1-C6 alkyl.

D in each occurrence, independently is a bond, an optionally substituted alkylene group, -(CH<sub>2</sub>)<sub>1</sub>C(O)O(CH<sub>2</sub>)<sub>1</sub>-, -(CH<sub>2</sub>)<sub>1</sub>NHC(O)(CH<sub>2</sub>)<sub>1</sub>-, -(CH<sub>2</sub>)<sub>1</sub>C(O)NH(CH<sub>2</sub>)<sub>1</sub>-, -(CH<sub>2</sub>)<sub>1</sub>C(O)O(CH<sub>2</sub>)<sub>1</sub>-, -(CH<sub>2</sub>)<sub>1</sub>OC(O)(CH<sub>2</sub>)<sub>1</sub>-, -(CH<sub>2</sub>)<sub>1</sub>CH=N(CH<sub>2</sub>)<sub>1</sub>-, -(CH<sub>2</sub>)<sub>1</sub>N=CH(CH<sub>2</sub>)<sub>1</sub>-, -(CH<sub>2</sub>)<sub>1</sub>NH(CH<sub>2</sub>)<sub>1</sub>-, -(CH<sub>2</sub>)<sub>1</sub>S-(CH<sub>2</sub>)<sub>1</sub>-, -(CH<sub>2</sub>)<sub>1</sub>O(CH<sub>2</sub>)<sub>1</sub> or -(CH<sub>2</sub>)<sub>1</sub>C(O)(CH<sub>2</sub>)<sub>1</sub>-. 30

Z in each occurrence, independently is a bond, an optionally substituted alkylene group, -S-, -O- or -NH-.

i and j in each occurrence, independently is 0, 1, 2, 3 or 4. In one embodiment i and j in each occurrence, independently is 0, 1 or 2. In a particular embodiment, i is 0. In another particular embodiment, j is 2.

k is a positive integer from 1 to 20. In one embodiment, k is a positive integer from 1 to 12. In another embodiment, k is a positive integer from 1 to 6.

l is 0 or a positive integer from 1 to 20. In one embodiment, l is 0 or a positive integer from 1 to 12. In another embodiment, l is 0 or a positive integer from 1 to 6.

n and m in each occurrence independently is 0 or a positive integer. In one embodiment, n and m in each occurrence independently is 0 to 18. In another embodiment, n and m in each occurrence independently is 0 to 12. In yet another embodiment, n and m are in each occurrence independently is 0 to 6.

s is a positive integer from 1 to 6.

q is a positive integer from 1 to 3.

D in each occurrence, independently is a bond, an optionally substituted alkylene group, -(CH<sub>2</sub>)<sub>1</sub>C(O)O(CH<sub>2</sub>)<sub>h</sub>-,

-(CH<sub>2</sub>)<sub>1</sub>NHC(O)(CH<sub>2</sub>)<sub>h</sub>-, -(CH<sub>2</sub>)<sub>1</sub>OC(O)(CH<sub>2</sub>)<sub>h</sub>-, -(CH<sub>2</sub>)<sub>1</sub>CH=N(CH<sub>2</sub>)<sub>h</sub>-, -(CH<sub>2</sub>)<sub>1</sub>N=CH(CH<sub>2</sub>)<sub>h</sub>-, -(CH<sub>2</sub>)<sub>1</sub>NH(CH<sub>2</sub>)<sub>h</sub>-, -(CH<sub>2</sub>)<sub>1</sub>S-(CH<sub>2</sub>)<sub>h</sub>-, -(CH<sub>2</sub>)<sub>1</sub>O(CH<sub>2</sub>)<sub>h</sub> or -(CH<sub>2</sub>)<sub>1</sub>C(O)(CH<sub>2</sub>)<sub>h</sub>-. 5

Z in each occurrence, independently is a bond, an optionally substituted alkylene group, -S-, -O- or -NH-. In a particular embodiment, Z is a single bond.

i and j in each occurrence, independently is 0, 1, 2, 3 or 4.

10 In one embodiment i and j in each occurrence, independently is 0, 1 or 2. In a particular embodiment, i is 0. In another particular embodiment, j is 2.

k is a positive integer from 1 to 20. In one embodiment, k is a positive integer from 1 to 12. In another embodiment, k is a 15 positive integer from 1 to 6.

1 is 0 or a positive integer from 1 to 20, and when D is -(CH<sub>2</sub>)<sub>1</sub>NHC(O)(CH<sub>2</sub>)<sub>h</sub>-, -(CH<sub>2</sub>)<sub>1</sub>OC(O)(CH<sub>2</sub>)<sub>h</sub>-, -(CH<sub>2</sub>)<sub>1</sub>S-(CH<sub>2</sub>)<sub>h</sub>-, or -(CH<sub>2</sub>)<sub>1</sub>O(CH<sub>2</sub>)<sub>h</sub>-, l is not 0. In one embodiment, l is 0 or a positive integer from 1 to 12. In 20 another embodiment, l is 0 or a positive integer from 1 to 6.

h is 0 or a positive integer from 1 to 20. When Z is not a bond and D is -(CH<sub>2</sub>)<sub>1</sub>C(O)O(CH<sub>2</sub>)<sub>h</sub>-, -(CH<sub>2</sub>)<sub>1</sub>C(O)NH(CH<sub>2</sub>)<sub>h</sub>-, -(CH<sub>2</sub>)<sub>1</sub>C(O)O(CH<sub>2</sub>)<sub>h</sub>-, -(CH<sub>2</sub>)<sub>1</sub>NH(CH<sub>2</sub>)<sub>h</sub>-, -(CH<sub>2</sub>)<sub>1</sub>S-(CH<sub>2</sub>)<sub>h</sub>-, or -(CH<sub>2</sub>)<sub>1</sub>O(CH<sub>2</sub>)<sub>h</sub>-, h is not 0. In one embodiment, h is 0 or a positive integer from 1 to 12. In another embodiment, h is 0 or a positive integer from 1 to 6. In another embodiment, h is 0.

In certain other embodiments R is:



50 R<sub>1</sub> and R<sub>2</sub> in each occurrence, independently is -H, -OH, a C1-C10 alkyl group or a tert-butyl group; A is -NHC(O)- or -C(O)O- and B is a bond or a C1-C24 alkylene, and i and j are 0, 1, 2, 3 or 4.

55 In other certain embodiments, the present invention is directed to macromolecular antioxidants represented by a structural formula selected from Structural Formulas 1-6, wherein R is:



wherein:

$D^a$ , for each occurrence, is independently  $-\text{C}(\text{O})\text{NR}_d$ ,  $-\text{NR}_d\text{C}(\text{O})-$ ,  $-\text{NR}_d-$ ,  $-\text{CR}_d=\text{N}-$ ,  $-\text{C}(\text{O})-$ ,  $-\text{C}(\text{O})\text{O}-$ ,  $-\text{OC}(\text{O})-$ ,  $-\text{O}-$ ,  $-\text{S}-$ ,  $-\text{C}(\text{O})\text{OC}(\text{O})-$  or a bond. In certain other embodiments  $D^a$  is  $-\text{C}(\text{O})\text{O}-$ ,  $-\text{OC}(\text{O})-$ ,  $-\text{C}(\text{O})\text{NH}-$ ,  $-\text{NHC}(\text{O})-$ ,  $-\text{NH}-$ ,  $-\text{O}-$  or  $-\text{C}(\text{O})-$ . In certain other embodiments,  $D^a$  is  $-\text{NH}-$ ,  $-\text{C}(\text{O})\text{NH}-$  or  $-\text{NHC}(\text{O})-$ . Optionally,  $D^a$  is not  $-\text{C}(\text{O})\text{O}-$ ,  $-\text{OC}(\text{O})-$ ,  $-\text{O}-$  or  $-\text{NH}-$ . In various embodiments, the present invention relates to a compound of Structural Formula I and the attendant definitions, wherein  $D^a$  is  $-\text{OC}(\text{O})-$ . In another embodiment,  $D^a$  is  $-\text{C}(\text{O})\text{O}-$ . In another embodiment,  $D^a$  is  $-\text{C}(\text{O})\text{NH}-$ . In another embodiment,  $D^a$  is  $-\text{NHC}(\text{O})-$ . In another embodiment,  $D^a$  is  $-\text{NH}-$ . In another embodiment,  $D^a$  is  $-\text{CH}=\text{N}-$ . In another embodiment,  $D^a$  is  $-\text{C}(\text{O})-$ . In another embodiment,  $D^a$  is  $-\text{O}-$ . In another embodiment,  $D^a$  is  $-\text{C}(\text{O})\text{OC}(\text{O})-$ . In another embodiment,  $D^a$  is a bond.

Each  $R_d$  is independently  $-\text{H}$  or optionally substituted alkyl. In certain other embodiments  $R_d$  is  $-\text{H}$  or an alkyl group. In certain other embodiments  $R_d$  is  $-\text{H}$  or a C<sub>1</sub>-C<sub>10</sub> alkyl group. In certain other embodiments  $R_d$  is  $-\text{H}$ .

$R_c$  and  $R_c'$  are independently H or an optionally substituted alkyl. In one embodiment,  $R_c$  and  $R_c'$  are H. In another embodiment, one of  $R_c$  and  $R_c'$  is H and the other is an optionally substituted alkyl. More specifically, the alkyl is a C<sub>1</sub>-C<sub>10</sub> alkyl. Even more specifically, the alkyl is a C<sub>10</sub> alkyl.

$R^a$ , for each occurrence, is independently an optionally substituted alkyl, optionally substituted aryl, optionally substituted alkoxy carbonyl, optionally substituted ester,  $-\text{OH}$ ,  $-\text{NH}_2$ , or  $-\text{SH}$ . In certain other embodiments, each  $R^a$  is independently an optionally substituted alkyl or optionally substituted alkoxy carbonyl. In certain other embodiment

each  $R^a$  is independently an alkyl or alkoxy carbonyl. In certain other embodiments each  $R^a$  is independently a C<sub>1</sub>-C<sub>6</sub> alkyl or a C<sub>1</sub>-C<sub>6</sub> alkoxy carbonyl. In certain other embodiments each  $R^a$  is independently tert-butyl or propoxy carbonyl. In certain other embodiments each  $R^a$  is independently an alkyl group. In certain embodiments each  $R^a$  is independently a bulky alkyl group. Suitable examples of bulky alkyl groups include butyl, sec-butyl, tert-butyl, 2-propyl, 1,1-dimethylhexyl, and the like. In certain embodiments each  $R^a$  is tert-butyl. In certain embodiments at least one  $R^a$  adjacent to the  $-\text{OH}$  group is a bulky alkyl group (e.g., butyl, sec-butyl, tert-butyl, 2-propyl, 1,1-dimethylhexyl, and the like). In certain other embodiments both  $R^a$  groups adjacent to  $-\text{OH}$  are bulky alkyl groups (e.g., butyl, sec-butyl, tert-butyl, 2-propyl, 1,1-dimethylhexyl, and the like). In another embodiment, both  $R^a$  groups are tert-butyl. In another embodiment, both  $R^a$  groups are tert-butyl adjacent to the OH group.

$R^b$ , for each occurrence, is independently H or optionally substituted alkyl. In certain embodiment,  $R^b$  is H.

Each  $n'$  and  $m'$  are independently integers from 0 to 18. In another embodiment,  $n'$  and  $m'$  in each occurrence, independently is 0 to 12. In yet another embodiment,  $n'$  and  $m'$  in each occurrence, independently is 0 to 6. In certain embodiments each  $n'$  and  $m'$  are independently integers from 0 to 2. In a specific embodiment,  $n'$  is 0. In another specific embodiment,  $m'$  is an integer from 0 to 2. In another specific embodiment,  $n'$  is 0 and  $m'$  is 2.

Each  $p'$  is independently an integer from 0 to 4. In certain embodiments, each  $p'$  is independently an integer from 0 to 2. In certain embodiments,  $p'$  is 2.

In one embodiment the first antioxidants which are suitable for use in the compositions and methods of the present invention are represented by:



In an additional embodiment, for formulas 1-6 R is:



89

n and m in each occurrence, independently is 0 or a positive integer. In one embodiment, n and m in each occurrence, independently is 0 to 18. In another embodiment, n and m in each occurrence, independently is 0 to 12. In yet another embodiment, n and m in each occurrence, independently is 0 to 6.

i and j in each occurrence, independently is 0, 1, 2, 3 or 4. In one embodiment, i and j in each occurrence, independently is 0, 1 or 2. In a particular embodiment, i is 0. In another particular embodiment, j is 2.

Z' in each occurrence, independently is  $-\text{C}(\text{O})\text{O}-$ ,  $-\text{OC}(\text{O})-$ ,  $-\text{C}(\text{O})\text{NH}-$ ,  $-\text{NHC}(\text{O})-$ ,  $-\text{NH}-$ ,  $-\text{CH}=\text{N}-$ ,  $-\text{C}(\text{O})-$ ,  $-\text{O}-$ ,  $-\text{S}-$ ,  $-\text{C}(\text{O})\text{OC}(\text{O})-$  or a bond. In one embodiment, Z' is  $-\text{C}(\text{O})\text{O}-$ . In another embodiment, Z' is  $-\text{OC}(\text{O})-$ . In yet another embodiment, Z' is  $-\text{C}(\text{O})\text{NH}-$ . In yet another embodiment, Z' is  $-\text{NHC}(\text{O})-$ . In yet another embodiment, Z' is  $-\text{NH}-$ . In yet another embodiment, Z' is  $-\text{CH}=\text{N}-$ . In yet another embodiment, Z' is  $-\text{C}(\text{O})-$ . In yet another embodiment, Z' is  $-\text{O}-$ . In yet another embodiment, Z' is  $-\text{S}-$ .

In yet another embodiment, Z' is  $-\text{C}(\text{O})\text{OC}(\text{O})-$ . In yet another embodiment, Z' is a bond.

R' in each occurrence, independently is C1-C6 alkyl,  $-\text{OH}$ ,  $-\text{NH}_2$ ,  $-\text{SH}$ , an optionally substituted aryl, an ester or



wherein at least one R' adjacent to the  $-\text{OH}$  group is an optionally substituted bulky alkyl group (e.g., butyl, sec-butyl, tert-butyl, 2-propyl, 1,1-dimethylhexyl, and the like).

R'1 in each occurrence, independently is C1-C6 alkyl, an optionally substituted aryl, an optionally substituted aralkyl,  $-\text{OH}$ ,  $-\text{NH}_2$ ,  $-\text{SH}$ , or C1-C6 alkyl ester wherein at least one R1 adjacent to the  $-\text{OH}$  group is a bulky alkyl group (e.g., butyl, sec-butyl, tert-butyl, 2-propyl, 1,1-dimethylhexyl, and the like)).

R'2 in each occurrence, independently is C1-C6 alkyl, an optionally substituted aryl, an optionally substituted aralkyl,  $-\text{OH}$ ,  $-\text{NH}_2$ ,  $-\text{SH}$ , or ester.

X' in each occurrence, independently is  $-\text{C}(\text{O})\text{O}-$ ,  $-\text{OC}(\text{O})-$ ,  $-\text{C}(\text{O})\text{NH}-$ ,  $-\text{NHC}(\text{O})-$ ,  $-\text{NH}-$ ,  $-\text{CH}=\text{N}-$ ,  $-\text{C}(\text{O})-$ ,  $-\text{O}-$ ,  $-\text{S}-$ ,  $-\text{C}(\text{O})\text{OC}(\text{O})-$  or a bond. In one embodiment X' is  $-\text{C}(\text{O})\text{O}-$ . In another embodiment X' is  $-\text{OC}(\text{O})-$ . In yet another embodiment X' is  $-\text{C}(\text{O})\text{NH}-$ . In yet another embodiment X' is  $-\text{NHC}(\text{O})-$ . In yet another embodiment X' is  $-\text{NH}-$ . In yet another embodiment X' is  $-\text{CH}=\text{N}-$ . In yet another embodiment X' is  $-\text{C}(\text{O})-$ . In

90

yet another embodiment X' is  $-\text{O}-$ . In yet another embodiment X' is  $-\text{S}-$ . In yet another embodiment X' is  $-\text{C}(\text{O})\text{OC}(\text{O})-$ . In yet another embodiment X' is a bond.

M' is H, an optionally substituted aryl, C1-C20 linear or branched alkyl chain with or without any functional group anywhere in the chain, or



o is 0 or a positive integer. Preferably o is 0 to 18. More preferably o is 0 to 12. Even more preferably o is 0 to 6.

In yet another embodiment, for formulas 1-6 R is:



R'2 is C1-C6 alkyl,  $-\text{OH}$ ,  $-\text{NH}_2$ ,  $-\text{SH}$ , aryl, aralkyl, ester, or



wherein at least one R'2 is  $-\text{OH}$ , and the values and preferred values for the remainder of the variables for R are as described immediately above.

In yet another embodiment, the present invention relates to a compound of formula 1-6, wherein M is



Wherein p is 0, 1, 2, 3 or 4; and the values and preferred values for the remainder of the variables are as described above for formulas 1-6.

Specific examples of first macromolecular antioxidants which are suitable for use in the compositions and methods of the present invention, for example, high molecular weight dimers, and tetramers etc., are shown below.



-continued



-continued



-continued



The values and preferred values for the variables are as described above.

In another embodiment, the first antioxidants which are suitable for use in the compositions and methods of the present invention are represented by a structural formula selected from 7a, 7b, 8a and 8b:



$R_3$  and  $R_4$  in each occurrence, independently is C1-C16 alkyl,  $-\text{O}-(\text{C1-C16 alkyl})$ ,  $-\text{NH(aryl)}$ ,  $-\text{NH}_2$ ,  $-\text{OH}$ , or  $-\text{SH}$ .

$p$  in each occurrence, independently is an integer equal to or greater than 2.

Specific examples of polymers which are useful in the compositions methods of the present invention include:

In one embodiment antioxidants suitable for use in the methods and compositions of the present invention include compounds represented by Structural Formula I:



99

wherein:

R and R' are independently H or optionally substituted alkyl and at least one of R and R' is H;

Z is  $-\text{C}(\text{O})\text{NR}^c-$ ,  $-\text{NR}^c\text{C}(\text{O})-$ ,  $-\text{NR}^c-$ ,  $-\text{CR}^c=\text{N}-$ ,  $-\text{C}(\text{O})-$ ,  $-\text{C}(\text{O})\text{O}-$ ,  $-\text{OC}(\text{O})-$ ,  $-\text{O}-$ ,  $-\text{S}-$ ,  $-\text{C}(\text{O})\text{OC}(\text{O})-$  or a bond;

$\text{R}^c$  is independently H or optionally substituted alkyl;

$\text{R}^a$ , for each occurrence, is independently an optionally substituted alkyl, optionally substituted aryl, optionally substituted alkoxy carbonyl, optionally substituted ester, <sup>10</sup>  $-\text{OH}$ ,  $-\text{NH}_2$ ,  $-\text{SH}$ ;

100

$\text{R}^b$ , for each occurrence, is independently H or optionally substituted alkyl;

s, for each occurrence, is independently an integer from 0 to 4; and

m and n, for each occurrence, are independently integers from 0 to 6.

In one embodiment antioxidants suitable for use in the methods and compositions of the present invention include compounds represented by Structural Formula II:



20

wherein:

R and R' are independently H or optionally substituted alkyl and at least one of R and R' is H;

$\text{R}^a$ , for each occurrence, is independently an optionally substituted alkyl, optionally substituted aryl, optionally substituted alkoxy carbonyl, optionally substituted ester,  $-\text{OH}$ ,  $-\text{NH}_2$ , or  $-\text{SH}$ ;

$\text{R}^b$ , for each occurrence, is independently H or optionally substituted alkyl.

s, for each occurrence, is independently an integer from 0 to 4; and

m, for each occurrence, is independently an integer from 0 to 6.

In one embodiment antioxidants suitable for use in the methods and compositions of the present invention include compounds represented by Structural Formula III:



III

wherein R and R' are independently H or optionally substituted alkyl and at least one of R and R' is H.

In one embodiment antioxidants suitable for use in the methods and compositions of the present invention include a compound A represented by the following structural formula:



(A)

## 101

In one embodiment antioxidants suitable for use in the methods and compositions of the present invention include a compound B represented by the following structural formula:



In one embodiment, the first antioxidants which are suitable for use in the compositions and methods of the present invention include antioxidant polymers which comprises at least one repeat unit selected from:



X is  $-\text{O}-$ ,  $-\text{NH}-$  or  $-\text{S}-$ . Each  $\text{R}_{10}$  is independently an optionally substituted C1-C10 alkyl group, an optionally substituted aryl group, and optionally substituted alkoxy group, an optionally substituted carbonyl group, an optionally substituted alkoxy carbonyl group, an optionally substituted aryloxycarbonyl group,  $-\text{OH}$ ,  $-\text{SH}$  or  $-\text{NH}_2$  or two  $\text{R}_{10}$  groups on adjacent carbon atoms join together to form an optionally substituted aromatic ring or an optionally substituted carbocyclic or heterocyclic non-aromatic ring.  $q$  is an integer from 0 to 2.  $\text{R}_{12}$  is a bulky alkyl group substituent bonded to a ring carbon atom adjacent (ortho) to a ring carbon atom substituted with an  $-\text{OH}$ ,  $-\text{SH}$  or  $-\text{NH}_2$  group. In certain embodiments,  $\text{R}_{12}$  is a bulky alkyl group substituent bonded to a ring carbon atom meta or para to a ring carbon atom substituted with an  $-\text{OH}$ ,  $-\text{SH}$  or  $-\text{NH}_2$  group.

In certain embodiments, the first antioxidants which are suitable for use in the compositions and methods of the present invention include antioxidant polymers which comprises at least one repeat unit selected from:



$\text{R}_{13}$  is an aryl group. In certain embodiments, the aryl group is adjacent (or ortho) to an  $-\text{OH}$ ,  $-\text{SH}$  or  $-\text{NH}_2$  group. In

## 102

certain embodiments, the aryl group is adjacent (or ortho) to an  $-\text{OH}$  group. In certain embodiments, the aryl group is meta or para to an  $-\text{OH}$ ,  $-\text{SH}$  or  $-\text{NH}_2$  group. Each  $\text{R}_{10}$  is



independently an optionally substituted C1-C10 alkyl group, an optionally substituted aryl group, and optionally substituted alkoxy group, an optionally substituted carbonyl group, an optionally substituted alkoxy carbonyl group, an optionally substituted aryloxycarbonyl group,  $-\text{OH}$ ,  $-\text{SH}$  or  $-\text{NH}_2$  or two  $\text{R}_{10}$  groups on adjacent carbon atoms join together to form an optionally substituted aromatic ring or an optionally substituted carbocyclic or heterocyclic non-aromatic ring.  $q$  is an integer from 0 to 2.  $\text{R}_{12}$  is a bulky alkyl group substituent bonded to a ring carbon atom adjacent (ortho) to a ring carbon atom substituted with an  $-\text{OH}$  group.

In certain embodiments, the  $-\text{OH}$  groups in the structures in the two immediately preceding paragraphs may be replaced with  $-\text{SH}$  or  $-\text{NH}_2$ .

In one embodiment, the first antioxidants which are suitable for use in the compositions and methods of the present invention include a macromonomer represented by the following structural formula:



103

Each of R and R<sub>1</sub>-R<sub>8</sub> are independently —H, —OH, or a C1-C10 alkyl group. n is an integer from 0 to 24. R<sup>1</sup> is —H, optionally substituted C1-C20 alkyl or optionally substituted aryl group.

#### Stabilized Lubricant Oil Compositions

Lubricants, lubricant oils, mixtures thereof and compositions comprising lubricants and lubricant oils can be improved by the methods of the present invention, by contacting the lubricant, lubricant oil, mixtures thereof or composition comprising the lubricant or lubricant oil or mixtures thereof with antioxidants, additives and mixtures thereof as described herein.

As used here, the terms "lubricants" and "lubricant oils" can be used interchangeably. Examples of lubricants suitable for use in the compositions and methods of the present invention include, but are not limited to: i) petroleum based oils (Group I, II and III), ii) synthetic oils (Group IV) and iii) biolubricant oils (vegetable oils such as canola, soybean, corn oil etc.). Group I oils, as defined herein are solvent refined base oils. Group II oils, as defined herein are modern conventional base oils made by hydrocracking and early wax isomerization, or hydroisomerization technologies and have significantly lower levels of impurities than Group I oils. Group III oils, as defined herein are unconventional base oils. Groups I-III differ in impurities, and viscosity index as is shown in Kramer et al. "The Evolution of Base Oil Technology" *Turbine Lubrication in the 21<sup>st</sup> Century* ASTM STP #1407 W. R. Herguth and T. M. Wayne, Eds., American Society for Testing and Materials, West Conshohocken, Pa., 2001 the entire contents of which are incorporated herein by reference. Group IV oils as defined herein are "synthetic" lubricant oils, including for example, poly-alpha olefins (PAOs). Biolubricants as defined herein are lubricants which contain at least 51% biomaterial (see Scott Fields, Environmental Health Perspectives, volume 111, number 12, September 2003, the entire contents of which are incorporated herein by reference). Other examples of lubricant oils can be found in Melvyn F. Askew "Biolubricants-Market Data Sheet" IENICA, August 2004 (as part of the IENICA workstream of the IENICA-INFORRM project); Taylor et al. "Engine lubricant Trends Since 1990" paper accepted for publication in the Proceedings I. Mech. E. Part J, Journal of Engineering Tribology, 2005 (Vol. 219 p 1-16); and Desplanches et al. "Formulating Tomorrow's Lubricants" page 49-52 of 'The Paths to Sustainable Development, part of special report published in October 2003 by Total; the entire contents of each of which are incorporated herein by reference. Biolubricants are often but not necessarily, based on vegetable oils. Vegetable derived, for example, from rapeseed, sunflower, palm and coconut can be used as biolubricants. They can also be synthetic esters which may be partly derived from renewable resources. They can be made from a wider variety of natural sources including solid fats and low grade or waste materials such as tallow. Biolubricants in general offer rapid biodegradability and low environmental toxicity.

#### Additives

Examples of first additives suitable for use in the compositions and methods of the present invention, include but are not limited to, surface additives, performance enhancing additives and lubricant protective additives.

Surface additives: In certain embodiments of the present invention, surface additives can protect the surfaces that are lubricated from wear, corrosion, rust, and friction. Examples of these surface additives suitable for use in the compositions and methods of the present invention include, but are not limited to: (a) rust inhibitors, (b) corrosion inhibitors, (c) extreme pressure agents, (d) tackiness agents, (e) antiwear

104

agents, (f) detergents and dispersants, (g) compounded oil (like fat or vegetable oil to reduce the coefficient of friction without affecting the viscosity), (h) antimisting, (i) seal swelling agents and (j) biocides.

5 Performance Enhancing Additives: In certain embodiments of the present invention, performance enhancing additives improve the performance of lubricants. Examples of these performance enhancing additives suitable for use in the Compositions and methods of the present invention include, 10 but are not limited to: (a) pour-point depressants, (b) viscosity index modifiers (c) emulsifiers, and (d) demulsifiers.

Lubricant Protective Additives: In certain embodiments of the present invention, lubricant protective additives maintain the quality of oil from oxidation and other thermal degradation processes. Examples of these lubricant protective additives suitable for use in the compositions and methods of the present invention include, but are not limited to: (a) oxidation 15 inhibitors and (b) foam inhibitors.

#### Other Lubricant Additives

20 In certain embodiments, a second additive can be used in the compositions and methods of the present invention in combination with the first antioxidant and the first additive as described above. Examples of second additives suitable for use in the compositions and methods of the present invention include, 25 include but are not limited to, for example, dispersants, detergents, corrosion inhibitors, rust inhibitors, metal deactivators, antiwear and extreme pressure agents, antifoam agents, friction modifiers, seal swell agents, demulsifiers, viscosity index improvers, pour point depressants, and the like. See, for example, U.S. Pat. No. 5,498,809 for a description of useful lubricating oil composition additives, the disclosure of which is incorporated herein by reference in its entirety.

Dispersants: Examples of dispersants suitable for use in the 30 compositions and methods of the present invention include, but are not limited to: polybutenylsuccinic acid-amides, -imides, or -esters, polybutenylphosphonic acid derivatives, Mannich Base ashless dispersants, and the like.

Detergents: Examples of detergents suitable for use in the 35 compositions and methods of the present invention include, but are not limited to: metallic phenolates, metallic sulfonates, metallic salicylates, metallic phosphonates, metallic thiophosphonates, metallic thiopyrophosphonates, and the like.

40 Corrosion Inhibitors: Examples of corrosion inhibitors suitable for use in the compositions and methods of the present invention include, but are not limited to: phosphosulfurized hydrocarbons and their reaction products with an alkaline earth metal oxide or hydroxide, hydrocarbyl-thio-substituted derivatives of 1,3,4-thiadiazole, thiadiazole polysulphides and their derivatives and polymers thereof, thio and polythio sulphenamides of thiadiazoles such as those described in U.K. Patent Specification 1,560,830, and the like.

45 Rust Inhibitors: Examples of rust inhibitors suitable for use in the compositions and methods of the present invention include, but are not limited to: nonionic surfactants such as polyoxyalkylene polyols and esters thereof, anionic surfactants such as salts of alkyl sulfonic acids, and other compounds such as alkoxylated fatty amines, amides, alcohols and the like, including alkoxylated fatty acid derivatives treated with C9 to C16 alkyl-substituted phenols (such as the mono- and di-heptyl, octyl, nonyl, decyl, undecyl, dodecyl and tridecyl phenols).

50 Metal Deactivators: Metal deactivators as used herein, are the additives which form an inactive film on metal surfaces by complexing with metallic ions and reducing, for example, the

## 105

catalytic effect on metal gum formation and other oxidation. Examples of metal deactivators suitable for use in the compositions and methods of the present invention include, but are not limited to: N,N-disubstituted aminomethyl-1,2,4-triazoles, N,N-disubstituted aminomethyl-benzotriazoles, mixtures thereof, and the like.

Antiwear and Extreme Pressure Additives: Antiwear and extreme pressure additives, as used herein, react with metal surfaces to form a layer with lower shear strength than metal, thereby preventing metal to metal contact and reducing friction and wear. Examples of antiwear additives suitable for use in the compositions and methods of the present invention include, but are not limited to: sulfurized olefins, sulfurized esters, sulfurized animal and vegetable oils, phosphate esters, organophosphites, dialkyl alkylphosphonates, acid phosphates, zinc dialkyldithiophosphates, zinc diaryldithiophosphates, organic dithiophosphates, organic phosphorothiolates, organic thiophosphates, organic dithiocarbamates, dimercaptothiadiazole derivatives, mercaptobenzothiazole derivatives, amine phosphates, amine thiophosphates, amine dithiophosphates, organic borates, chlorinated paraffins, and the like.

Antifoam Agents: Examples of antifoam agents suitable for use in the compositions and methods of the present invention include, but are not limited to: polysiloxanes and the like.

Friction Modifiers: Examples of friction modifiers suitable for use in the compositions and methods of the present invention include, but are not limited to: fatty acid esters and amides, organic molybdenum compounds, molybdenum dialkylthiocarbamates, molybdenum dialkyl dithiophosphates, molybdenum dithiolates, copper oleate, copper salicylate, copper dialkyldithiophosphates, molybdenum disulfide, graphite, polytetrafluoroethylene, and the like.

Seal Swell Agents: Seal swell agents, as used herein, react chemically with elastomers to cause slight swell thus improving low temperature performance especially in, for example, aircraft hydraulic oil. Examples of seal swell agents suitable for use in the compositions and methods of the present invention include, but are not limited to: dioctyl sebacate, dioctyl adipate, dialkyl phthalates, and the like.

Demulsifiers: Demulsifiers, as used herein promote separation of oil and water in lubricants exposed to water. Examples of demulsifiers suitable for use in the compositions and methods of the present invention include, but are not limited to: the esters described in U.S. Pat. Nos. 3,098,827 and 2,674,619 incorporated herein by reference.

Viscosity Index Improvers: Examples of viscosity index improvers suitable for use in the compositions and methods of the present invention include, but are not limited to: olefin copolymers, dispersant olefin copolymers, polymethacrylates, vinylpyrrolidone/methacrylate-copolymers, polyvinylpyrrolidones, polybutanes, styrene-acrylate-copolymers, polyethers, and the like.

Pour Point Depressants: Pour point depressants as used herein reduce the size and cohesiveness of crystal structure resulting in low pour point and increased flow at low-temperatures. Examples of pour point depressants suitable for use in the compositions and methods of the present invention include, but are not limited to: polymethacrylates, alkylated naphthalene derivatives, and the like.

## Other Antioxidants and Stabilizers

In certain embodiments, a second antioxidant or a stabilizer can be used in the compositions and methods of the present invention in combination with the first antioxidant and the first additive and optionally the second additive as described above. Examples of second antioxidants suitable

## 106

for use in the compositions and methods of the present invention include, include but are not limited to:

1. Amine Antioxidants
  - 1.1. Alkylated Diphenylamines, for example octylated diphenylamine; styrenated diphenylamine; mixtures of mono- and dialkylated tert-butyl-tert-octyl diphenylamines; and 4,4'-dicumyldiphenylamine.
  - 1.2. Phenyl Naphthylamines, for example N-phenyl-1-naphthylamine; N-phenyl-2-naphthylamine; tert-octylated N-phenyl-1-naphthylamine.
  - 1.3. Derivatives of para-Phenylenediamine, for example N,N'-diisopropyl-p-phenylenediamine; N,N'-di-sec-butyl-p-phenylenediamine; N,N'-bis(1,4-dimethylpentyl)-p-phenylenediamine; N,N'-bis(1-ethyl-3-methylpentyl)-p-phenylenediamine; N,N'-bis(1-methylheptyl)-p-phenylenediamine; N,N'-diphenyl-p-phenylenediamine; N,N'-di-(naphthyl-2)-p-phenylenediamine; N-isopropyl-N'-phenyl-p-phenylenediamine; N-(1,3-dimethylbutyl)-N'-phenyl-p-phenylenediamine; N-(1-methylheptyl)-N'-phenyl-p-phenylenediamine; N-cyclohexyl-N'-phenyl-p-phenylenediamine; N,N'-dimethyl-N,N'-di-sec-butyl-p-phenylenediamine.
  - 1.4. Phenothiazines, for example phenothiazine; 2-methylphenothiazine; 3-octylphenothiazine; 2,8-dimethylphenothiazine; 3,7-dimethylphenothiazine; 3,7-diethylphenothiazine; 3,7-dibutylphenothiazine; 3,7-diethylphenothiazine; 2,8-diethylphenothiazine; 2,8-diethylphenothiazine.
  - 1.5. Dihydroquinolines, for example 2,2,4-trimethyl-1,2-dihydroquinoline or a polymer thereof
2. Phenolic Antioxidants
  - 2.1. Alkylated monophenols, for example 2,6-di-tert-butyl-4-methylphenol; 2,6-di-tert-butylphenol; 2-tert-butyl-4,6-dimethylphenol; 2,6-di-tert-butyl-4-ethylphenol; 2,6-di-tert-butyl-4-n-butylphenol; 2,6-di-tert-butyl-4-isobutylphenol; 2,6-di-tert-butyl-4-sec-butylphenol; 2,6-di-tert-butyl-4-octadecylphenol; 2,6-di-tert-butyl-4-nonylphenol; 2,6-dicyclopentyl-4-methylphenol; 2-( $\alpha$ -methylcyclohexyl)-4,6-dimethylphenol; 2,6-di-octadecyl-4-methylphenol; 2,4,6-tricyclohexylphenol; 2,6-di-tert-butyl-4-methoxymethylphenol; 2,6-di-tert-butyl-4-dimethylaminomethylphenol; o-tert-butylphenol.
  - 2.2. Alkylated hydroquinones, for example 2,6-di-tert-butyl-4-methoxyphenol; 2,5-di-tert-butylhydroquinone; 2,5-di-tert-amylhydroquinone; 2,6-di-phenyl-4-octadecylox-phenol.
  - 2.3. Hydroxylated thiodiphenyl ethers, for example 2,2'-thiobis(6-tert-butyl-4-methyl-phenol); 2,2'-thiobis(4-octylphenol); 4,4'-thiobis(6-tert-butyl-3-methylphenol); 4,4'-thiobis(6-tert-butyl-2-methylphenol).
  - 2.4. Alkylidenebisphenols, for example 2,2'-methylenebis(6-tert-butyl-4-methylphenol); 2,2'-methylenebis(6-tert-butyl-4-ethylphenol); 2,2'-methylenebis(4-methyl-6-( $\alpha$ -methylcyclohexyl)phenol); 2,2'-methylenebis(4-methyl-6-cyclohexylphenol); 2,2'-methylenebis(6-nonyl-4-methylphenol); 2,2'-methylenebis(4,6-di-tert-butylphenol); 2,2'-ethylidenebis(6-tert-butyl-4-isobutylphenol); 2,2'-methylenebis[6- $\alpha$ -methylbenzyl)-4-nonylphenol]; 2,2'-methylenebis[6-( $\alpha$ , $\alpha$ -dimethylbenzyl)-4-nonylphenol]; 4,4'-methylenebis(2,6-di-tert-butylphenol); 4,4'-methylenebis(6-tert-butyl-2-methylphenol); 1,1-bis(5-tert-butyl-4-hydroxy-2-methylphenyl)butane; 2,6-di(3-tert-butyl-5-methyl-2-hydroxybenzyl)-4-methylphenol; 1,1,3-tris(5-tert-butyl-4-hydroxy-2-methylphenyl)-3-n-dodecylmercaptobutane; ethylene glycol bis[3,3-bis(3'-tert-butyl-4'-hydroxylphenyl)butyrate]; di(3-tert-butyl-4-hydroxy-5-methylphenyl)

- dicyclopentadiene; di[2-(3'-tert-butyl-2'-hydroxy-5'-methylbenzyl)-6-tert-butyl-4-methylphenyl]terephthalate.
- 2.5. Benzyl compounds, for example 1, 3,5-tris(3,5-di-tert-butyl-4-hydroxybenzyl)-2,4,6-trimethylbenzene; di(3,5-di-tert-butyl-4-hydroxybenzyl)sulfide; 3,5-di-tert-butyl-4-hydroxybenzylmercaptoacetic acid isoctyl ester; bis(4-tert-butyl-3-hydroxy-2,6-dimethylbenzyl)dithiophthalate; 1,3,5-tris(3,5-di-tert-butyl-4-hydroxybenzyl)isocyanurate; 1,3,5-tris(4-tert-butyl-3-hydroxy-2,6-dimethylbenzyl)isocyanurate; 3,5-di-tert-butyl-4-hydroxybenzylphosphonic acid dioctadecyl ester; 3,5-di-tert-butyl-4-hydroxybenzylphosphonic acid monoethyl ester calcium salt.
- 2.6. Acylaminophenols, for example 4-hydroxylauric acid anilide; 4-hydroxystearic acid anilide; 2,4-bis-octylmercapto-6-(3,5-di-tert-butyl-4-hydroxyaniline)-s-triazine; N-(3,5-di-tert-butyl-4-hydroxyphenyl)carbamic acid octyl ester.
- 2.7. Esters of  $\beta$ -(3,5-di-tert-butyl-4-hydroxyphenyl)propionic acid with mono- or polyhydric alcohols, e.g. with methanol; octadecanol; 1,6-hexanediol; neopentyl glycol; thiidiethylene glycol; diethylene glycol; triethylene glycol; pentaerythritol; tris(hydroxyethyl)isocyanurate; and di(hydroxyethyl)oxalic acid diamide.
- 2.8. Esters of  $\beta$ -(5-tert-butyl-4-hydroxy-3-methylphenyl)propionic acid with mono- or polyhydric alcohols, e.g. with methanol; octadecanol; 1,6-hexanediol; neopentyl glycol; thiidiethylene glycol; diethylene glycol; triethylene glycol; pentaerythritol; tris(hydroxyethyl)isocyanurate; and di(hydroxyethyl)oxalic acid diamide.
- 2.9. Amides of  $\beta$ -(3,5-di-tert-butyl-4-hydroxyphenyl)propionic acid, e.g., N,N'-di(3,5-di-tert-butyl-4-hydroxyphenyl-propionyl)hexamethylenediamine; N,N'-di(3,5-di-tert-butyl-4-hydroxyphenylpropionyl)trimethylenediamine; N,N'-di(3,5-di-tert-butyl-4-hydroxyphenylpropionyl)hydrazine.
3. Sulfurized organic compounds, for example aromatic, alkyl, or alkenyl sulfides and polysulfides; sulfurized olefins; sulfurized fatty acid esters; sulfurized ester olefins; sulfurized oils; esters of  $\beta$ -thiodipropionic acid; sulfurized Diels-Alder adducts; sulfurized terpene compounds; and mixtures thereof.
4. Organo-borate compounds, for example alkyl- and aryl-(and mixed alkyl, aryl) substituted borates.
5. Phosphite and phosphate antioxidants, for example alkyl- and aryl-(and mixed alkyl, aryl) substituted phosphites, and alkyl- and aryl- (and mixed alkyl, aryl) substituted dithiophosphates such as O,O,S-trialkyl dithiophosphates, O,O,S-triaryldithiophosphates and dithiophosphates having mixed substitution by alkyl and aryl groups, phosphorothionyl sulfide, phosphorus-containing silane, polyphenylene sulfide, amine salts of phosphinic acid and quinone phosphates.
6. Copper compounds, for example copper dihydrocarbyl thio- or dithiophosphates, copper salts of synthetic or natural carboxylic acids, copper salts of alkenyl carboxylic acids or anhydrides such as succinic acids or anhydrides, copper dithiocarbamates, copper sulphonates, phenates, and acetylacetones. The copper may be in cuprous ( $Cu^I$ ) or cupric ( $Cu^{II}$ ) form.
7. Zinc dithiodiphosphates, for example zinc dialkyldithiophosphates, diphenyldialkyldithiophosphates, and di(alkylphenyl)dithiophosphates.
- In one embodiment, the compositions for use in the methods of the present invention, include but are not limited to:
- a. a first antioxidant (in the concentration range, from about 0.0001% to about 50%, from about 0.0005% to about 20%,

- from about 0.005% to about 10%, from about 0.05% to about 5% or from about 0.01% to about 1%) with a first additive selected from the group comprising a surface additive, a performance enhancing additive and a lubricant performance additive, for example, in amounts of from about 0.0005% to about 50%, from about 0.0001% to about 20%, from about 0.005% to about 10%, from about 0.05% to about 5% or from about 0.01% to about 1% by weight, based on the weight of lubricant to be stabilized.
- 10 b. the first antioxidant and the first additive as described in a. and a second additive, for example, in concentrations of from about 0.0001% to about 50% by weight, about 0.0005% to about 20% by weight, about 0.001% to about 10% by weight, from about 0.01% to about 5% by weight, from about 0.05% to about 1% by weight from about 0.1% to about 1% by weight based on the overall weight of the lubricant to be stabilized.
- 15 c. the first antioxidant and the first additive as described in a. and optionally the second additive as described in b. and a second antioxidant, for example, Irganox<sup>®</sup> 1010, Irganox<sup>®</sup> 1330, Irganox<sup>®</sup> 1076, Irganox<sup>®</sup> 5057 and Irganox<sup>®</sup> 1135 in the concentration range, from about 0.0001% to about 50%, from about 0.0005% to about 20%, from about 0.005% to about 10%, from about 0.05% to about 5% or from about 0.01% to about 1%) by weight, based on the weight of lubricant to be stabilized.
- 20 The term "alkyl" as used herein means a saturated straight-chain, branched or cyclic hydrocarbon. When straight-chained or branched, an alkyl group is typically C1-C8, more typically C1-C6; when cyclic, an alkyl group is typically C3-C12, more typically C3-C7 alkyl ester. Examples of alkyl groups include methyl, ethyl, n-propyl, iso-propyl, n-butyl, sec-butyl and tert-butyl and 1,1-dimethylhexyl.
- 25 The term "alkoxy" as used herein is represented by —OR<sup>\*\*</sup>, wherein R<sup>\*\*</sup> is an alkyl group as defined above.
- 30 The term "carbonyl" as used herein is represented by —C(=O)R<sup>\*\*</sup>, wherein R<sup>\*\*</sup> is an alkyl group as defined above.
- 35 The term "alkoxycarbonyl" as used herein is represented by —C(=O)OR<sup>\*\*</sup>, wherein R<sup>\*\*</sup> is an alkyl group as defined above.
- 40 The term "aromatic group" includes carbocyclic aromatic rings and heteroaryl rings. The term "aromatic group" may be used interchangeably with the terms "aryl", "aryl ring" "aromatic ring", "aryl group" and "aromatic group".
- 45 Carbocyclic aromatic ring groups have only carbon ring atoms (typically six to fourteen) and include monocyclic aromatic rings such as phenyl and fused polycyclic aromatic ring systems in which a carbocyclic aromatic ring is fused to one or more aromatic rings (carbocyclic aromatic or heteroaromatic). Examples include 1-naphthyl, 2-naphthyl, 1-anthracyl and 2-anthracyl. Also included within the scope of the term "carbocyclic aromatic ring", as it is used herein, is a group in which an aromatic ring is fused to one or more non-aromatic rings (carbocyclic or heterocyclic), such as in an indanyl, phthalimidyl, naphthimidyl, phenanthridinyl, or tetrahydronaphthyl, where the radical or point of attachment is on the aromatic ring.
- 50 The term "heteroaryl", "heteroaromatic", "heteroaryl ring", "heteroaryl group" and "heteroaromatic group", used alone or as part of a larger moiety as in "heteroaralkyl" refers to heteroaromatic ring groups having five to fourteen members, including monocyclic heteroaromatic rings and polycyclic aromatic rings in which a monocyclic aromatic ring is fused to one or more other aromatic ring (carbocyclic or heterocyclic). Heteroaryl groups have one or more ring heteroatoms. Examples of heteroaryl groups include 2-furanyl,

## 109

3-furanyl, N-imidazolyl, 2-imidazolyl, 4-imidazolyl, 5-imidazolyl, 3-isoxazolyl, 4-isoxazolyl, 5-isoxazolyl, oxadiazolyl, oxadiazolyl, 2-oxazolyl, 4-oxazolyl, 5-oxazolyl, N-pyrazolyl, 3-pyrazolyl, 4-pyrazolyl, 5-pyrazolyl, N-pyrrolyl, 2-pyrrolyl, 3-pyrrolyl, 2-pyridyl, 3-pyridyl, 4-pyridyl, 2-pyrimidinyl, 4-pyrimidinyl, 5-pyrimidinyl, 3-pyridazinyl, 4-pyridazinyl, 2-thiazolyl, 4-thiazolyl, 5-thiazolyl, triazolyl, tetrazolyl, 2-thienyl, 3-thienyl, carbazolyl, benzothienyl, benzofuranyl, indolyl, quinolinyl, benzothiazole, benzoazole, benzimidazolyl, isoquinolinyl and isoindolyl. Also included within the scope of the term "heteroaryl", as it is used herein, is a group in which an aromatic ring is fused to one or more non-aromatic rings (carbocyclic or heterocyclic), where the radical or point of attachment is on the aromatic ring.

The term non-aromatic heterocyclic group used alone or as part of a larger moiety refers to non-aromatic heterocyclic ring groups having three to fourteen members, including monocyclic heterocyclic rings and polycyclic rings in which a monocyclic ring is fused to one or more other non-aromatic carbocyclic or heterocyclic ring or aromatic ring (carbocyclic or heterocyclic). Heterocyclic groups have one or more ring heteroatoms, and can be saturated or unsaturated. Examples of heterocyclic groups include piperidinyl, piperizinyl, pyrrolidinyl, pyrazolidinyl, imidazolidinyl, tetrahydroquinolinyl, inodolinyl, isoindolinyl, tetrahydrofuranyl, oxazolidinyl, thiazolidinyl, dioxolanyl, dithiolanyl, tetrahydropyranyl, dihydropyranyl, azepanyl and azetidinyl.

The term "heteroatom" means nitrogen, oxygen, or sulfur and includes any oxidized form of nitrogen and sulfur, and the quaternized form of any basic nitrogen. Also the term "nitrogen" includes a substitutable nitrogen of a heteroaryl or non-aromatic heterocyclic group. As an example, in a saturated or partially unsaturated ring having 0-3 heteroatoms selected from oxygen, sulfur or nitrogen, the nitrogen may be N (as in 3,4-dihydro-2H-pyrrolyl), NH (as in pyrrolidinyl) or NR" (as in N-substituted pyrrolidinyl), wherein R" is a suitable substituent for the nitrogen atom in the ring of a non-aromatic nitrogen-containing heterocyclic group, as defined below.

As used herein the term non-aromatic carbocyclic ring as used alone or as part of a larger moiety refers to a non-aromatic carbon containing ring which can be saturated or unsaturated having three to fourteen atoms including monocyclic and polycyclic rings in which the carbocyclic ring can be fused to one or more non-aromatic carbocyclic or heterocyclic rings or one or more aromatic (carbocyclic or heterocyclic) rings.

An optionally substituted aryl group as defined herein may contain one or more substitutable ring atoms, such as carbon or nitrogen ring atoms. Examples of suitable substituents on a substitutable ring carbon atom of an aryl group include halogen (e.g., —Br, Cl, I and F), —OH, C1-C4 alkyl, C1-C4 haloalkyl, —NO<sub>2</sub>, C1-C4 alkoxy, C1-C4 haloalkoxy, —CN, —NH<sub>2</sub>, C1-C4 alkylamino, C1-C4 dialkylamino, —C(O)NH<sub>2</sub>, —C(O)NH(C1-C4 alkyl), —C(O)(C1-C4 alkyl), —OC(O)(C1-C4 alkyl), —OC(O)(aryl), —OC(O)(substituted aryl), —OC(O)(aralkyl), —OC(O)(substituted aralkyl), —NHC(O)H, —NHC(O)(C1-C4 alkyl), —C(O)N(C1-C4 alkyl)<sub>2</sub>, —NHC(O)O—(C1-C4 alkyl), —C(O)OH, —C(O)O—(C1-C4 alkyl), —NHC(O)NH<sub>2</sub>, —NHC(O)NH(C1-C4 alkyl), —NHC(O)N(C1-C4 alkyl)<sub>2</sub>, —NH—C(=NH)NH<sub>2</sub>, —SO<sub>2</sub>NH<sub>2</sub>, —SO<sub>2</sub>NH(C1-C3alkyl), —SO<sub>2</sub>N(C1-C3alkyl)<sub>2</sub>, NHSO<sub>2</sub>H, NHSO<sub>2</sub>(C1-C4 alkyl) and optionally substituted aryl. Preferred substituents on aryl groups are as defined throughout the specification. In certain embodiments aryl groups are unsubstituted.

## 110

Examples of suitable substituents on a substitutable ring nitrogen atom of an aryl group include C1-C4 alkyl, NH<sub>2</sub>, C1-C4 alkylamino, C1-C4 dialkylamino, —C(O)NH<sub>2</sub>, —C(O)NH(C1-C4 alkyl), —C(O)(C1-C4 alkyl), —CO<sub>2</sub>R\*\*, —C(O)C(O)R\*\*, —C(O)CH<sub>3</sub>, —C(O)OH, —C(O)O—(C1-C4 alkyl), —SO<sub>2</sub>NH<sub>2</sub>, —SO<sub>2</sub>NH(C1-C3 alkyl), —SO<sub>2</sub>N(C1-C3alkyl)<sub>2</sub>, NHSO<sub>2</sub>H, NHSO<sub>2</sub>(C1-C4 alkyl), —C(=S)NH<sub>2</sub>, —C(=S)NH(C1-C4 alkyl), —C(=S)N(C1-C4 alkyl)<sub>2</sub>, —C(=NH)—N(H)<sub>2</sub>, —C(=NH)—NH(C1-C4 alkyl) and —C(=NH)—N(C1-C4 alkyl)<sub>2</sub>,

An optionally substituted alkyl group or non-aromatic carbocyclic or heterocyclic group as defined herein may contain one or more substituents. Examples of suitable substituents for an alkyl group include those listed above for a substitutable carbon of an aryl and the following: =O, =S, =NNHR\*\*, =NN(R\*\*)<sub>2</sub>, =NNHC(O)R\*\*, =NNHCO<sub>2</sub>(alkyl), =NNHSO<sub>2</sub>(alkyl), =NR\*\*, Spiro cycloalkyl group or fused cycloalkyl group. R\*\* in each occurrence, independently is —H or C<sub>1</sub>-C<sub>6</sub> alkyl. Preferred substituents on alkyl groups are as defined throughout the specification. In certain embodiments optionally substituted alkyl groups are unsubstituted.

A "spiro cycloalkyl" group is a cycloalkyl group which shares one ring carbon atom with a carbon atom in an alkylene group or alkyl group, wherein the carbon atom being shared in the alkyl group is not a terminal carbon atom.

Without wishing to be bound by any theory or limited to any mechanism it is believed that macromolecular antioxidants and polymeric macromolecular antioxidants of the present invention exploit the differences in activities (ks, equilibrium constant) of, for example, homo- or hetero-type antioxidant moieties. Antioxidant moieties include, for example, hindered phenolic groups, unhindered phenolic groups, aminic groups and thioester groups, etc. of which there can be one or more present in each macromolecular antioxidant molecule. As used herein a homo-type antioxidant macromolecule comprises antioxidant moieties which are all same, for example, hindered phenolic, —OH groups. As used herein a hetero-type antioxidant macromolecule comprises at least one different type of moiety, for example, hindered phenolic and aminic groups in the one macromolecule.

This difference in activities can be the result of, for example, the substitutions on neighboring carbons or the local chemical or physical environment (for example, due to electrochemical or stereochemical factors) which can be due in part to the macromolecular nature of molecules.

In one embodiment of the present invention, a series of macromolecular antioxidant moieties of the present invention with different chemical structures can be represented by W1H, W2H, W3H, . . . to WnH. In one embodiment of the present invention, two types of antioxidant moieties of the present invention can be represented by: W1H and W2H. In certain embodiments W1H and W2H can have rate constants of k1 and k2 respectively. The reactions involving these moieties and peroxy radicals can be represented as:



## 111

where ROO. is a peroxy radical resulting from, for example, initiation steps involving oxidation activity, for example:



In one particular embodiment of the present invention  $k_1 \gg k_2$  in equations (1) and (2). As a result, the reactions would take place in such a way that there is a decrease in concentration of W1. free radicals due their participation in the regeneration of active moiety W2H in the molecule according equation (5):



This transfer mechanism may take place either in intra- or inter-molecular macromolecules. The transfer mechanism (5) could take place between moieties residing on the same macromolecule (intra-type) or residing on different macromolecules (inter-type).

In certain embodiments of the present invention, the antioxidant properties described immediately above (equation 5) of the macromolecular antioxidants and polymeric macromolecular antioxidants of the present invention result in advantages including, but not limited to:

- a) Consumption of free radicals W1. according to equation (5) can result in a decrease of reactions of W1. with hydroperoxides and hydrocarbons (RH).
- b) The regeneration of W1H provides extended protection of materials. This is a generous benefit to sacrificial type of antioxidants that are used today. Regeneration of W1H assists in combating the oxidation process. The increase in the concentration of antioxidant moieties W1H (according to equation 5) extends the shelf life of materials.

In certain embodiments of the present invention, the following items are of significant interest for enhanced antioxidant activity in the design of the macromolecular antioxidants and polymeric macromolecular antioxidants of the present invention:

- a) The activity of proposed macromolecular antioxidant is dependent on the regeneration of W1H in equation (5) either through inter- or intra-molecular activities involving homo- or hetero-type antioxidant moieties.
- b) Depending on the rates constants of W1H and W2H it is possible to achieve performance enhancements by many multiples and not just incremental improvements.

In certain embodiments of the present invention, more than two types of antioxidant moieties with different rate constants are used in the methods of the present invention.

In certain embodiments, the present invention pertains to the use of the disclosed compositions to improve materials, such as lubricants, lubricant oils, compositions comprising lubricants and lubricant oils and mixtures thereof.

In certain embodiments, as defined herein improving a material means inhibiting oxidation of an oxidizable material.

For purposes of the present invention, a method of "inhibiting oxidation" is a method that inhibits the propagation of a free radical-mediated process. Free radicals can be generated by heat, light, ionizing radiation, metal ions and some proteins and enzymes. Inhibiting oxidation also includes inhibiting reactions caused by the presence of oxygen, ozone or another compound capable of generating these gases or reactive equivalents of these gases.

As used herein the term "oxidizable material" is any material which is subject to oxidation by free-radicals or oxidative reaction caused by the presence of oxygen, ozone or another

## 112

compound capable of generating these gases or reactive equivalents thereof. In particular the oxidizable material is a lubricant or a mixture of lubricants.

In certain other embodiments, as defined herein improving a material means inhibiting oxidation, as well as improving performance and/or increasing the quality of a material, such as, a lubricant, lubricant oil, composition comprising a lubricant or lubricant oil or mixtures thereof. Increasing the quality of a material includes reducing friction and wear, increasing viscosity, resistance to corrosion, aging or contamination, etc. In certain embodiments, improving means that the lubricant is more resistant to degradation due to the presence of oxygen, temperature, pressure, water, metal species and other contributing factors to degradation. In certain embodiments, additive as described herein help to promote the shelf life of these oils. In certain embodiments the stability of the lubricants is directly related to their performance. That is the lubricant will not perform well if the lubricant has been degraded. In certain embodiments the performance of the lubricants is related to the additives. That is if antioxidant and additives are used they will result in an improvement in the stability and performance of the lubricants.

A lubricant, as defined herein is a substance (usually a liquid) introduced between two moving surfaces to reduce the friction and wear between them. Lubricant can be used in, for example, automotive engines, hydraulic fluids with transmission oils and the like. In addition to automotive and industrial applications, lubricants are used for many other purposes, including bio-medical applications (e.g. lubricants for artificial joints), grease, aviation lubricants, turbine engine lubricants, compressor oils, power transformer oils, automatic transmission fluids, metal working fluids, gear oils, sexual lubricants and others.

Non-liquid lubricants include grease, powders (dry graphite, PTFE, Molybdenum disulfide, etc.), teflon tape used in plumbing, air cushion and others.

The entire teachings of each of the following applications are incorporated herein by reference:

40 Provisional Patent Application No. 60/632,893, filed Dec. 3, 2004, Title: Process For The Synthesis Of Polyalkylphenol Antioxidants, by Suizhou Yang, et al;

PCT Application No.: PCT/US2005/044021, filed Dec. 2, 2005, Title: Process For The Synthesis Of Polyalkylphenol Antioxidants, by Suizhou Yang, et al;

Provisional Patent Application No. 60/633,197, filed Dec. 3, 2004, Title: Synthesis Of Sterically Hindered Phenol Based Macromolecular Antioxidants, by Ashish Dhawan, et al.;

50 PCT Application No.: PCT/US2005/044022, filed Dec. 2, 2005, Title: Synthesis Of Sterically Hindered Phenol Based Macromolecular Antioxidants, by Ashish Dhawan, et al.;

Provisional Patent Application No. 60/633,252, filed Dec. 3, 2004, Title: One Pot Process For Making Polymeric Antioxidants, by Vijayendra Kumar, et al.;

PCT Application No.: PCT/US2005/044023, filed Dec. 2, 2005, Title: One Pot Process For Making Polymeric Antioxidants, by Vijayendra Kumar, et al.;

60 Provisional Patent Application No. 60/633,196, filed Dec. 3, 2004, Title: Synthesis Of Aniline And Phenol-Based Macromonomers And Corresponding Polymers, by Rajesh Kumar, et al.;

PCT Application No.: PCT/US2005/044019, filed Dec. 2, 2005, Title: Synthesis Of Aniline And Phenol-Based Macromonomers And Corresponding Polymers, by Rajesh Kumar, et al.;

113

Patent application Ser. No. 11/184,724, filed Jul. 19, 2005, Title: Anti-Oxidant Macromonomers And Polymers And Methods Of Making And Using The Same, by Ashok L. Cholli;

Patent application Ser. No. 11/184,716, filed Jul. 19, 2005, Title: Anti-Oxidant Macromonomers And Polymers And Methods Of Making And Using The Same, by Ashok L. Cholli;

Provisional Patent Application No. 60/655,169, filed Feb. 22, 2005, Title: Nitrogen And Hindered Phenol Containing Dual Functional Macromolecules: Synthesis And Their Antioxidant Performances In Organic Materials, by Rajesh Kumar, et al.

Provisional Patent Application No. 60/655,638, filed Mar. 25, 2005, Title: Alkylated Macromolecular Antioxidants And Methods Of Making, And Using The Same, by Rajesh Kumar, et al.

Provisional Patent Application No. 60/731,125, filed Oct. 27, 2005, Title: Macromolecular Antioxidants And Polymeric Macromolecular Antioxidants, by Ashok L. Cholli, et al.

Provisional Patent Application No. 60/731,021, filed Oct. 27, 2005, Title:, Title: Macromolecular Antioxidants Based On Sterically Hindered Phenols And Phosphites, by Ashok L. Cholli, et al.

Provisional Patent Application No. 60/731,325, filed Oct. 27, 2005, Title:, Title: Stabilized Polyolefin Composition, by Kumar, Rajesh, et al.

Patent application Ser. No. 11/040,193, filed Jan. 21, 2005, Title: Post-Coupling Synthetic Approach For Polymeric Antioxidants, by Ashok L. Choll, et al.;

Patent Application No.: PCT/US2005/001948, filed Jan. 21, 2005, Title: Post-Coupling Synthetic Approach For Polymeric Antioxidants, by Ashok L. Cholli et al.;

Patent Application No.: PCT/US2005/001946, filed Jan. 21, 2005, Title: Polymeric Antioxidants, by Ashok L. Choll, et al.;

Patent Application No.: PCT/US03/10782, filed Apr. 4, 2003, Title: Polymeric Antioxidants, by Ashok L. Choll, et al.;

Patent application Ser. No. 10/761,933, filed Jan. 21, 2004, Title: Polymeric Antioxidants, by Ashish Dhawan, et al.;

Patent application Ser. No. 10/408,679, filed Apr. 4, 2003, Title: Polymeric Antioxidants, by Ashok L. Choll, et al.; Tertiary Butoxy Derivatives of Phenol. (Jan Pospisil and Ludek Taimr). (1964), 2 pp. CS 111291

A New Synthesis of aryl tert-butyl Ethers. Masada, Hiromitsu; Oishi, Yutaka. Fac. Eng., Kanazawa Univ., Kanazawa, Japan. Chemistry Letters (1978), (1), 57-8.

Simple Synthesis of the tert-butyl Ether of Phenol. Ol'dekop, Yu. A.; Maier, N. A.; Erdman, A. A.; Shirokii, V. L.; Zubrejchuk, Z. P.; Beresnevich, L. B. Inst. Fiz.-Org. Khim., Minsk, USSR. Zhurnal Obshchei Khimii (1980), 50(2), 475-6.

New Method for the Williamson Ether Synthesis Using tert-alkyl Halides in Nonpolar Solvents. Masada, Hiromitsu; Mikuchi, Fumio; Doi, Yasuo; Hayashi, Akira Dep. Chem. Chem. Eng., Kanazawa Univ., Kanazawa, Japan. Nippon Kagaku Kaishi (1995), (2), 164-6.

New Heterogeneous Williamson Synthesis of Ethers Using tert-alkyl Substrates. Masada, Hiromitsu; Doi, Yasuo; Mikuchi, Fumio; Keiko, Kigoshi. Faculty Eng., Kanazawa Univ., Kanazawa, Japan. Nippon Kagaku Kaishi (1996), (3), 275-82.

Preparation of Aromatic Tertiary Ethers. Tanaka, Masato; Reddy, Nagaveri Prabacal. (Agency of Industrial Sciences and Technology, Japan). Jpn. Kokai Tokkyo Koho (1999), 3 pp. JP 080063.

114

Preparation of Aromatic Ethers. Watanabe, Makoto; Koie, Yasuyuki. (Tosoh Corp., Japan). Jpn. Kokai Tokkyo Koho (1999), 10 pp. JP 11158103.

o-Alkylated phenols. Firth, Bruce E.; Rosen, Terry J. (UOP Inc., USA). U.S. Pat. No. 4,447,657 (1984), 4 pp.

2-Tert-Butyl-4-alkoxy- and -4-hydroxyphenols. Firth, Bruce E.; Rosen, Terry J. (UOP Inc., USA). U.S. Pat. No. 4,465, 871 (1984), 4 pp.

Conversion of Alkyl Phenyl Ether to Alkylphenol. Klicker, James D. (Borg-Warner Corp., USA). U.S. Pat. No. 4,283, 572 (1981), 3 pp.

O. N. Tsevktov, K. D. Kovenev, *Int. J. Chem. Eng.* 6 (1966), 328.

15 Sartori Giovanni, Franca Bigi et al., *Chem. Ind.* (London), 1985 (22) 762-763.

V. A. Koshchii, Ya. B. Kozlikovskii, A. A Matyusha, *Zh. Org. Khim.* 24(7), 1988, 1508-1512.

Gokul K. Chandra, M. M. Sharma, *Catal. Lett.* 19(4), 1993, 309-317.

Sakthivel, Ayyamperumal; Saritha, Nellutla; Selvam, Parasuraman, *Catal. Lett.* 72(3), 2001, 225-228.

V. Quaschning, J. Deutsch, P. Druska, H. J. Niclas and E. Kemnitz. *J. Catal.* 177 (1998), p. 164.

25 S. K. Badamali, S. Sakthivel and P. Selvam. *Catal. Today* 63 (2000), p. 291.

A. Heidekum, M. A. Hamm and F. Hoelderich. *J. Catal.* 188 (1999), p. 230.

30 Y. Kamitori, M. Hojo, R. Matsuda, T. Izumi and S. Tsukamoto. *J. Org. Chem.* 49 (1984), p. 4165.

E. Armengol, A. Corma, H. Garcia and J. Primo. *Appl. Catal. A* 149 (1997), p. 411.

J. M. Lalancette, M. J. Fournier and R. Thiffault. *Can. J. Chem.* 52 (1974), p. 589.

Japanese Patent No. JP 145002980, 1970.

Japanese Patent No. 44028850, 1969.

Japanese Patent No. 44024274, 1969.

## EXEMPLIFICATION

### Example 1

45 A commercial lubricant oil (example Castrol GTX 5W30) which comprises additives, was added to a known amount of a first antioxidant as cdescribed above.

The commercial lubricant oil alone was tested versus the commercial lubricant oil with the added antioxidant, using Passenger Car Motor Oil (PMCO) TEOST MHT test (ASTM D78097-05 test) performed at SWRI, Antonio Tex.

55 Test conditions include 285° C. for 24 hours, airflow, the deposit on the rod was then tested.

The deposit on the metal strip for the control sample was 46 mg, while for the sample containing the antioxidant was 18 mg. The difference of 28.1 mg was due to 1% of the antioxidant. The smaller deposit on the metal strip indicates the superior performance of the lubricant oil in combination with an antioxidant

60 While this invention has been particularly shown and described with references to preferred embodiments thereof, it will be understood by those skilled in the art that various changes in form and details may be made therein without departing from the scope of the invention encompassed by the appended claims.

## 115

What is claimed is:

1. A lubricant composition, consisting essentially of:
  - a) a lubricant or a mixture of lubricants;
  - b) an antioxidant component including a first antioxidant represented by the following structural formula:



10  
15

and  
20  
25  
30  
35  
40  
45  
50

- c) at least one first additive selected from the group consisting of

- i) a surface additive;
- ii) a performance enhancing additive; and
- iii) a lubricant protective additive;

wherein the concentration of the first antioxidant is between about 0.05% to about 5% by weight of the lubricant composition and the concentration of the first additive is between about 0.05% and about 5% by weight of the lubricant composition.

2. The lubricant composition of claim 1, wherein the first additive is a surface additive selected from the group consisting of (a) rust inhibitors, (b) corrosion inhibitors, (c) extreme pressure agents, (d) tackiness agents, (e) antiwear agents, (f) detergents and dispersants and (g) compounded oil.

3. The lubricant composition of claim 1, wherein the first additive is a performance enhancing additive selected from the group consisting of (a) pour-point depressants, (b) viscosity index modifiers, (c) emulsifiers, and (d) demulsifiers.

4. The lubricant composition of claim 1, wherein the additive is a lubricant protective additive selected from the group consisting of (a) oxidation inhibitors and (b) foam inhibitors.

5. The lubricant composition of claim 1, wherein the antioxidant component further includes a second antioxidant selected from the group consisting of: amine antioxidants, phenolic antioxidants, sulfurized organic compounds, organo-borate compounds, phosphite and phosphate antioxidants, copper compounds, and zinc dithiophosphates.

6. The lubricant composition of claim 1, wherein the lubricant is selected from the group consisting of petroleum based oils, synthetic oils and biolubricant oils.

## 116

7. A method of forming a lubricant composition, comprising the step of combining a lubricant or mixture of lubricants to form a lubricant composition consisting essentially of:
  - a) an antioxidant component including a first antioxidant represented by the following structural formula:



10  
15

- and  
20  
25  
30  
35  
40  
45  
50
- b) at least one first additive selected from the group consisting of:

- i) a surface additive;
- ii) a performance enhancing additive; and
- iii) a lubricant protective additive,

to thereby form a lubricant composition, wherein the concentration of the first antioxidant is between about 0.05% to about 5% by weight of the lubricant composition and the concentration of the first additive is between about 0.05% and about 5% by weight of the lubricant composition.

8. The method of claim 7, wherein the first additive is a surface additive selected from the group consisting of (a) rust inhibitors, (b) corrosion inhibitors, (c) extreme pressure agents, (d) tackiness agents, (e) antiwear agents, (f) detergents and dispersants and (g) compounded oil.

9. The method of claim 7, wherein the first additive is a performance enhancing additive selected from the group consisting of (a) pour-point depressants, (b) viscosity index modifiers, (c) emulsifiers, and (d) demulsifiers.

10. The method of claim 7, wherein the additive is a lubricant protective additive selected from the group consisting of (a) oxidation inhibitors and (b) foam inhibitors.

11. The method of claim 7, wherein the antioxidant component further includes a second antioxidant selected from the group consisting of: amine antioxidants, phenolic antioxidants, sulfurized organic compounds, organo-borate compounds, phosphite and phosphate antioxidants, copper compounds and zinc dithiophosphates.

12. The method of claim 7, wherein the lubricant is selected from the group consisting of petroleum based oils, synthetic oils and biolubricant oils.

\* \* \* \* \*